



US006218059B1

(12) **United States Patent**  
**Aylward et al.**

(10) **Patent No.:** **US 6,218,059 B1**  
(b4) **Date of Patent:** **Apr. 17, 2001**

(54) **TOUGH REFLECTIVE IMAGE DISPLAY MATERIAL**

(75) Inventors: **Peter T. Aylward**, Hilton; **Robert P. Bourdelais**, Pittsford; **Alphonse D. Camp**, Rochester, all of NY (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **09/470,806**

(22) Filed: **Dec. 22, 1999**

(51) **Int. Cl.<sup>7</sup>** ..... **G03C 1/79**; G03C 1/765; G03C 11/14

(52) **U.S. Cl.** ..... **430/11**; 430/14; 430/432; 430/531; 430/534; 430/536; 430/538; 430/961

(58) **Field of Search** ..... 430/536, 538, 430/534, 531, 496, 11, 14, 432, 961

(56) **References Cited**

U.S. PATENT DOCUMENTS

3,777,608 12/1973 Kopf et al. ..... 83/517

|           |        |                         |           |
|-----------|--------|-------------------------|-----------|
| 4,912,333 | 3/1990 | Roberts et al. ....     | 250/487.1 |
| 5,141,085 | 8/1992 | Maier et al. ....       | 264/45.3  |
| 5,212,053 | 5/1993 | McSweeney et al. ....   | 430/503   |
| 5,393,652 | 2/1995 | Marui ....              | 430/533   |
| 5,422,175 | 6/1995 | Ito et al. ....         | 428/304.4 |
| 5,866,282 | 2/1999 | Bourdelaire et al. .... | 430/536   |
| 5,888,643 | 3/1999 | Aylward et al. ....     | 430/536   |
| 5,888,714 | 3/1999 | Bourdelaire et al. .... | 430/536   |
| 5,902,720 | 5/1999 | Haydock et al. ....     | 430/536   |
| 6,020,116 | 2/2000 | Camp et al. ....        | 430/536   |
| 6,030,742 | 2/2000 | Bourdelaire et al. .... | 430/536   |

*Primary Examiner*—Richard L. Schilling

(74) *Attorney, Agent, or Firm*—Paul A. Leipold

(57)

**ABSTRACT**

This invention relates to a photographic element comprising at least one photosensitive layer, and a base material comprising an upper and lower biaxially oriented polymer sheet separated by a paper sheet, wherein said base material has a thickness of greater than 254 micrometers, a stiffness of greater than 325 millinewtons in any direction, and an upper surface roughness of less than 0.45 micrometers at a spatial frequency of between 0.30 and 6.35 millimeters, and a transmission percent of less than 15 percent.

**18 Claims, 1 Drawing Sheet**





## TOUGH REFLECTIVE IMAGE DISPLAY MATERIAL

### FIELD OF THE INVENTION

This invention relates to photographic materials. In a preferred form it relates to base materials for photographic reflective display.

### BACKGROUND OF THE INVENTION

It is known in the art that photographic display materials are utilized for advertising, as well as decorative displays of photographic images. Since these display materials are used in advertising, the image quality of the display material is critical in expressing the quality message of the product or service being advertised. Further, a photographic display image needs to be high impact, as it attempts to draw consumer attention to the display material and the desired message being conveyed. Typical applications for display material include product and service advertising in public places such as airports, buses and sports stadiums, movie posters, and fine art photography. The desired attributes of a quality, high impact photographic display material are a slight blue density minimum, durability, sharpness, and flatness. Cost is also important, as display materials tend to be expensive compared with alternative display material technology, mainly lithographic images on paper. For display materials, traditional color paper is undesirable, as it suffers from a lack of durability for the handling, photoprocessing, and display of large format images.

In the formation of color paper it is known that the base paper has applied thereto a layer of polymer, typically polyethylene. This layer serves to provide waterproofing to the paper, as well as providing a smooth surface on which the photosensitive layers are formed. The formation of a suitably smooth surface is difficult, requiring great care and expense to ensure proper laydown and cooling of the polyethylene layers. The formation of a suitably smooth surface would also improve image quality, as the display material would have more apparent blackness, as the reflective properties of the improved base are more specular than the prior materials. As the whites are whiter and the blacks are blacker, there is more range in between and, therefore, contrast is enhanced. It would be desirable if a more reliable and improved surface could be formed at less expense.

Prior art photographic reflective papers comprise a melt extruded polyethylene layer which also serves as a carrier layer for optical brightener and other whitener materials as well as tint materials. It would be desirable if the optical brightener, whitener materials and tints, rather than being dispersed throughout the single layer of polyethylene could be concentrated nearer the surface of the layer where they would be more effective optically.

Prior art photographic reflective display materials have light sensitive silver halide emulsions coated directly onto a gelatin coated opacified polyester base sheet. Since the emulsion does not contain any materials to opacify the imaging element, white pigments such as BaSO<sub>4</sub> have been added to the polyester base sheet to provide an imaging element with both opacity and the desired reflection properties. Also, optical brighteners are added to the polyester base sheet to give the sheet a blue tint in the presence of an ultraviolet light source. The addition of the white pigments into the polyester sheet causes several manufacturing problems which can either reduce manufacturing efficiency or reduce image quality. The addition of white pigment to the polyester base causes manufacturing problems, such as die

lines and pigment agglomeration, which reduce the efficiency at which photographic display material can be manufactured. It would be desirable if the optical brightener, whitener materials and tints, rather than being dispersed throughout the polyester base sheet, could be concentrated nearer the surface where they would be more effective optically and improve manufacturing efficiency.

Prior art reflective photographic materials with a polyester base use a TiO<sub>2</sub> pigmented polyester base onto which light sensitive silver halide emulsions are coated. It has been proposed in WO 94/04961 to use opaque polyester containing 10% to 25% TiO<sub>2</sub> for a photographic support. The TiO<sub>2</sub> in the polyester gives the reflective display materials an undesirable opalescence appearance. The TiO<sub>2</sub> pigmented polyester also is expensive because the TiO<sub>2</sub> must be dispersed into the entire thickness, typically from 100 to 180 micrometers. This also gives the polyester support a slight yellow tint which is undesirable for a photographic display material. For use as a photographic display material, the polyester support containing TiO<sub>2</sub> must be tinted blue to offset the yellow tint of the polyester causing a loss in desirable whiteness and adding cost to the display material. It would be desirable if a reflective display support did not contain any TiO<sub>2</sub> in the base and TiO<sub>2</sub> could be concentrated near the light sensitive emulsion.

Prior art photographic display material uses polyester as a base for the support. Typically the polyester support is from 150 to 250 micrometers thick to provide the required stiffness. A thinner base material would be lower in cost and allow for roll-handling efficiency, as the rolls would weigh less and be smaller in diameter. It would be desirable to use a base material that had the required stiffness but was thinner to reduce cost and improve roll-handling efficiency.

### PROBLEM TO BE SOLVED BY THE INVENTION

There is a continuing need for tough scratch resistant display materials that are low in cost and provide superior whiteness and color saturation.

### SUMMARY OF THE INVENTION

It is an object of the invention to overcome disadvantages of prior reflective display materials.

It is another object to provide lower cost, high quality reflective display materials.

These and other objects of the invention are accomplished by a photographic element comprising at least one photosensitive layer, and a base material comprising an upper and lower biaxially oriented polymer sheet separated by a paper sheet, wherein said base material has a thickness of greater than 254 micrometers, a stiffness of greater than 325 millinewtons in any direction, and an upper surface roughness of less than 0.45 micrometers at a spatial frequency of between 0.30 and 6.35 millimeters, and a transmission percent of less than 15 percent.

### ADVANTAGEOUS EFFECT OF THE INVENTION

The invention provides improved reflective display materials that provide whiter whites and have higher durability compared with polymer materials. The reflective display materials further provide a wider contrast range and sharper images. The invention materials are lower in cost compared to polymer materials.

### BRIEF DESCRIPTION OF THE DRAWING

The FIGURE illustrates the D LogH characteristic curve of a photographic element of the invention.

## DETAILED DESCRIPTION OF THE INVENTION

The invention has numerous advantages over prior practices in the art. The invention provides a display material that is scratch resistant and low in cost, as the material is overlaminated in its preferred form. The material provides superior color reproduction, superior whiteness, and sharpness. The material is readily digital processible for image formation. The material provides superior maximum density without having significant fringing of edges and text. The product has superior color gamut and is able to reproduce a broader range of color. Furthermore, when the base element of this invention is combined with a superior digitally compatible emulsion, a synergistic benefit is obtained as the whites are whiter and the blacks are blacker, and both pictorial scenes and text can now be combined with extremely sharp edges without text fringing and rastering, as the base is very reflective. The laminated base material utilized in the invention has superior stiffness which enables a thinner overlaminated, thereby resulting in cost savings as well as reduced weight of the product for equivalent stiffness as compared with previous products.

The reflective display material of the invention has a whiter white than prior materials. Prior materials were somewhat yellow and had a higher minimum density, as there was a large quantity of white pigment in the polymer base sheet. Typically when a large quantity of white  $TiO_2$  is loaded into a paper base, it becomes somewhat yellowish rather than being the desired neutral reflective white. The display material of the invention provides sharper images, as they have higher accutance due to the efficient reflective layer on the upper surface of the biaxially oriented polyolefin sheet. There is a visual contrast improvement in the display material of the invention, as the lower density is lower than prior product and the upper amount of density has been visually increased. The display material has a more maximum black, as the reflective properties of the improved base are more specular than the prior materials. As the whites are whiter and the blacks are blacker, there is more range in between and, therefore, contrast is enhanced. These and other advantages will be apparent from the detailed description below.

The terms as used herein, "top", "upper", "emulsion side", and "face" mean the side or toward the side of the photographic member bearing the imaging layers. The terms "bottom", "lower side", and "back" mean the side or toward the side of the photographic member opposite from the side bearing the photosensitive imaging layers or developed image.

A preferred embodiment of this invention utilizes a paper sheet that has a basis weight of greater than 200 g/m<sup>2</sup>. Such a basis weight is highly desirable because it allows the more expensive overlaminated to be down gauged (thinner), resulting in significant cost savings. Furthermore, the heavier basis weight of the paper sheet provides a feel of high quality. A paper sheet with a thickness of between 170 and 230  $\mu m$  is the most desired. When these materials are used for signage in a display booth, its superior weight, thickness, and stiffness minimizes sag. In the preferred embodiment a photographic element of thickness between 325 and 650 millinewtons is desired, as the materials are stiffer providing a display material. The photographic element with the overlaminated becomes self-supporting.

High performing biaxially oriented polyolefin sheet may be utilized for the sheet on the topside of the laminated base of the invention. Microvoided composite biaxially oriented

sheets are a preferred embodiment because the voids provide opacity without the use of  $TiO_2$ . Microvoided composite oriented sheets are conveniently manufactured by coextrusion of the core and surface layers, followed by biaxial orientation, whereby voids are formed around void-initiating material contained in the core layer. Such composite sheets are disclosed in, for example, U.S. Pat. Nos. 4,377,616; 4,758,462 and 4,632,869.

The core of the preferred topside composite sheet should be from 15 to 95% of the total thickness of the sheet, preferably from 30 to 85% of the total thickness. The nonvoided skin(s) should thus be from 5 to 85% of the sheet, preferably from 15 to 70% of the thickness.

The density (specific gravity) of the topside composite sheet, expressed in terms of "percent of solid density" is calculated as follows:

$$\text{Composite Sheet Density}/\text{Polymer Density} \times 100 = \% \text{ of Solid Density}$$

should be between 45% and 100%, preferably between 67% and 100%. As the percent solid density becomes less than 67%, the topside composite sheet becomes less manufacturable due to a drop in tensile strength and it becomes more susceptible to physical damage.

The total thickness of the topside composite sheet can range from 12 to 100 micrometers, preferably from 20 to 70 micrometers. Below 20 micrometers, the microvoided sheets may not be thick enough to minimize any inherent non-planarity in the support and would be more difficult to manufacture. At thickness higher than 70 micrometers, little improvement in either surface smoothness or mechanical properties are seen, and so there is little justification for the further increase in cost for extra materials.

"Void" is used herein to mean devoid of added solid and liquid matter, although it is likely the "voids" contain gas. The void-initiating particles which remain in the finished packaging sheet core should be from 0.1 to 10 micrometers in diameter, preferably round in shape, to produce voids of the desired shape and size. The size of the void is also dependent on the degree of orientation in the machine and transverse directions. Ideally, the void would assume a shape that is defined by two opposed and edge contacting concave disks. In other words, the voids tend to have a lens-like or biconvex shape. The voids are oriented so that the two major dimensions are aligned with the machine and transverse directions of the sheet. The Z-direction axis is a minor dimension and is roughly the size of the cross diameter of the voiding particle. The voids generally tend to be closed cells, and thus there is virtually no path open from one side of the voided-core to the other side through which gas or liquid can traverse.

The void-initiating material may be selected from a variety of materials, and should be present in an amount of about 5-50% by weight based on the weight of the core matrix polymer. Preferably, the void-initiating material comprises a polymeric material. When a polymeric material is used, it may be a polymer that can be melt-mixed with the polymer from which the core matrix is made and be able to form dispersed spherical particles as the suspension is cooled down. Examples of this would include nylon dispersed in polypropylene, polybutylene terephthalate in polypropylene, or polypropylene dispersed in polyethylene terephthalate. If the polymer is preshaped and blended into the matrix polymer, the important characteristic is the size and shape of the particles. Spheres are preferred and they can be hollow or solid. These spheres may be made from cross-linked polymers which are members selected from the

group consisting of an alkenyl aromatic compound having the general formula  $\text{Ar}-\text{C}(\text{R})=\text{CH}_2$ , wherein Ar represents an aromatic hydrocarbon radical, or an aromatic halohydrocarbon radical of the benzene series and R is hydrogen or the methyl radical; acrylate-type monomers include monomers of the formula  $\text{CH}_2=\text{C}(\text{R}')-\text{C}(\text{O})(\text{OR})$  wherein R is selected from the group consisting of hydrogen and an alkyl radical containing from about 1 to 12 carbon atoms and R' is selected from the group consisting of hydrogen and methyl; copolymers of vinyl chloride and vinylidene chloride, acrylonitrile and vinyl chloride, vinyl bromide, vinyl esters having formula  $\text{CH}_2=\text{CH}(\text{O})\text{COR}$ , wherein R is an alkyl radical containing from 2 to 18 carbon atoms; acrylic acid, methacrylic acid, itaconic acid, citraconic acid, maleic acid, fumaric acid, oleic acid, vinylbenzoic acid; the synthetic polyester resins which are prepared by reacting terephthalic acid and dialkyl terephthalates or ester-forming derivatives thereof, with a glycol of the series  $\text{HO}(\text{CH}_2)_n\text{OH}$  wherein n is a whole number within the range of 2-10 and having reactive olefinic linkages within the polymer molecule, the above described polyesters which include copolymerized therein up to 20 percent by weight of a second acid or ester thereof having reactive olefinic unsaturation and mixtures thereof, and a cross-linking agent selected from the group consisting of divinylbenzene, diethylene glycol dimethacrylate, diallyl fumarate, diallyl phthalate and mixtures thereof.

Examples of typical monomers for making the crosslinked polymer include styrene, butyl acrylate, acrylamide, acrylonitrile, methyl methacrylate, ethylene glycol dimethacrylate, vinyl pyridine, vinyl acetate, methyl acrylate, vinylbenzyl chloride, vinylidene chloride, acrylic acid, divinylbenzene, acrylamidomethylpropane sulfonic acid, vinyl toluene, etc. Preferably, the cross-linked polymer is polystyrene or poly(methyl methacrylate). Most preferably, it is polystyrene and the cross-linking agent is divinylbenzene.

Processes well known in the art yield non-uniformly sized particles, characterized by broad particle size distributions. The resulting beads can be classified by screening the beads spanning the range of the original distribution of sizes. Other processes such as suspension polymerization, limited coalescence, directly yield very uniformly sized particles.

The void-initiating materials may be coated with agents to facilitate voiding. Suitable agents or lubricants include colloidal silica, colloidal alumina, and metal oxides such as tin oxide and aluminum oxide. The preferred agents are colloidal silica and alumina, most preferably, silica. The cross-linked polymer having a coating of an agent may be prepared by procedures well known in the art. For example, conventional suspension polymerization processes wherein the agent is added to the suspension is preferred. As the agent, colloidal silica is preferred.

The void-initiating particles can also be inorganic spheres, including solid or hollow glass spheres, metal or ceramic beads or inorganic particles such as clay, talc, barium sulfate, and calcium carbonate. The important thing is that the material does not chemically react with the core matrix polymer to cause one or more of the following problems: (a) alteration of the crystallization kinetics of the matrix polymer, making it difficult to orient, (b) destruction of the core matrix polymer, (c) destruction of the void-initiating particles, (d) adhesion of the void-initiating particles to the matrix polymer, or (e) generation of undesirable reaction products, such as toxic or high color moieties. The void-initiating material should not be photographically active or degrade the performance of the photographic element in which the biaxially oriented polyolefin film is utilized.

For the top biaxially oriented sheets on the polymer base toward the emulsion, suitable classes of thermoplastic polymers for the biaxially oriented sheet and the core matrix-polymer of the preferred composite sheet comprise polyolefins. Suitable polyolefins include polypropylene, polyethylene, polymethylpentene, polystyrene, polybutylene and mixtures thereof. Polyolefin copolymers, including copolymers of propylene and ethylene such as hexene, butene, and octene are also useful. Polypropylene is preferred, as it is low in cost and has desirable strength properties. The biaxially oriented sheets used in the invention contain an integral emulsion bonding layer which avoids the need for expensive priming coatings or energy treatments. The bonding layer used in the invention is a low density polyethylene skin on the biaxially oriented sheet. Gelatin based silver halide emulsion layers of the invention have been shown to adhere well to low density polyethylene. The integral bonding skin layer also serves as a carrier for the blue tints that correct for the native yellowness of the gelatin based silver halide image element. Concentrating the blue tints in the thin, skin layer reduces the amount of expensive blue tint materials when compared to prior art photographic papers that contain blue tint materials dispersed in a single thick layer of polyethylene.

The nonvoided skin layers of the top and bottom composite sheet can be made of the same polymeric materials as listed above for the core matrix. The composite sheet can be made with skin(s) of the same polymeric material as the core matrix, or it can be made with skin(s) of different polymeric composition than the core matrix. For compatibility, an auxiliary layer can be used to promote adhesion of the skin layer to the core.

The total thickness of the top most skin layer or exposed surface layer below the image layers should be between 0.20  $\mu\text{m}$  and 1.5  $\mu\text{m}$ , preferably between 0.5 and 1.0  $\mu\text{m}$ . Below 0.5  $\mu\text{m}$  any inherent non-planarity in the coextruded skin layer may result in unacceptable color variation. At skin thickness greater than 1.0  $\mu\text{m}$ , there is a reduction in the photographic optical properties such as image resolution. At thickness greater than 1.0  $\mu\text{m}$  there is also a greater material volume to filter for contamination such as clumps, poor color pigment dispersion, or contamination.

Addenda may be added to the topmost skin layer to change the color of the imaging element. For photographic use, a white base with a slight bluish tinge is preferred. The addition of the slight bluish tinge may be accomplished by any process which is known in the art including the machine blending of color concentrate prior to extrusion and the melt extrusion of blue colorants that have been pre-blended at the desired blend ratio. Colored pigments that can resist extrusion temperatures greater than 320° C. are preferred, as temperatures greater than 320° C. are necessary for coextrusion of the skin layer. Blue colorants used in this invention may be any colorant that does not have an adverse impact on the imaging element. Preferred blue colorants include Phthalocyanine blue pigments, Cromophthal blue pigments, Irgazin blue pigments, Irgalite organic blue pigments, and pigment Blue 60.

One detail of this invention is that a very thin coating (0.2 to 1.5  $\mu\text{m}$ ) on the surface immediately below the emulsion layer can be made by coextrusion and subsequent stretching in the width and length direction. It has been found that this layer is, by nature, extremely accurate in thickness and can be used to provide all the color corrections, which are usually distributed throughout the thickness of the sheet between the emulsion and the polymer base. This topmost layer is so efficient that the total colorants needed to provide

a correction are less than one-half the amount needed if the colorants are dispersed throughout thickness. Colorants are often the cause of spot defects due to clumps and poor dispersions. Spot defects, which decrease the commercial value of images, are improved with this invention because less colorant is used and high quality filtration to clean up the colored layer is much more feasible since the total volume of polymer with colorant is only typically 2 to 10 percent of the total polymer between the base polymer and the photosensitive layer.

The addition of  $TiO_2$  or other white pigment known in the art to a layer of the photographic element of this invention contributes to the optical performance of the top sheet. In a preferred embodiment of this invention, the  $TiO_2$  is placed in a skin layer of the top biaxially oriented polymer sheet between the voided layer and the light sensitive silver halide emulsion. The  $TiO_2$  is preferred because it adds to the sharpness of the image as well as contributes to the overall opacity and whiteness of the photographic element. Additional white pigment may be added to the tie layer that is used to adhere the biaxially oriented polymer sheet to the base substrate. In this case the pigments contributes to improved opacity and sharpness.

Addenda may be added to the biaxially oriented sheet of this invention so that when the biaxially oriented sheet is viewed from a surface, the imaging element emits light in the visible spectrum when exposed to ultraviolet radiation. Emission of light in the visible spectrum allows for the support to have a desired background color in the presence of ultraviolet energy. This is particularly useful when images are viewed under lighting that contains ultraviolet energy and may be used to optimize image quality for consumer and commercial applications. The selection of white pigment in the biaxially oriented polymer sheet is important when there is ultraviolet illumination of the photographic image. In some cases the anatase form of  $TiO_2$  is preferred because it absorbs less ultraviolet energy and provides greater illumination in the blue region. The use of  $BaSO_4$  as the primary white pigment is preferred because it has very low ultraviolet absorbency and therefore has enhanced visible blue light reflection, which make the display materials appear very white. In the case when superior sharpness is desired the rutile form of  $TiO_2$  is preferred.

Addenda known in the art to emit visible light in the blue spectrum are preferred. Consumers generally prefer a slight blue tint to white defined as a negative  $b^*$  compared to a white defined as a  $b^*$  within one  $b^*$  unit of zero.  $b^*$  is the measure of yellow/blue in CIE space. A positive  $b^*$  indicates yellow while a negative  $b^*$  indicates blue. The addition of addenda that emits in the blue spectrum allows for tinting the support without the addition of colorants, which would decrease the whiteness of the image. The preferred emission is between 1 and 5 delta  $b^*$  units. Delta  $b^*$  is defined as the  $b^*$  difference measured when a sample is illuminated ultraviolet light source and a light source without any significant ultraviolet energy. Delta  $b^*$  is the preferred measure to determine the net effect of adding an optical brightener to the top biaxially oriented sheet of this invention. Emissions less than 1  $b^*$  unit can not be noticed by most customers therefore it is not cost effective to add optical brightener to the biaxially oriented sheet. An emission greater than 5  $b^*$  units would interfere with the color balance of the prints making the whites appear too blue for most consumers.

A preferred addendum of this invention is an optical brightener. An optical brightener is colorless, fluorescent, organic compound that absorbs ultraviolet light and emits it as visible blue light. Examples include but are not limited to

derivatives of 4,4'-diaminostilbene-2,2'-disulfonic acid, coumarin derivatives such as 4-methyl-7-diethylaminocoumarin, 1-4-Bis(O-Cyanostyryl)Benzol and 2-Amino-4-Methyl Phenol.

The optical brightener may be added to any layer in the multilayer coextruded biaxially oriented polyolefin sheet. The preferred locations are adjacent to or in the top most surface layer of the biaxially oriented sheet. This allows for the efficient concentration of optical brightener which results in less optical brightener being used when compared to traditional photographic supports. When the desired weight % loading of the optical brightener begins to approach the concentration at which the optical brightener migrates to the surface of the support forming crystals in the imaging layer, the addition of optical brightener into the layer adjacent to the exposed layer is preferred. When optical brightener migration is a concern as with light sensitive silver halide imaging systems, the preferred exposed layer comprised polyethylene. In this case, the migration from the layer adjacent to the exposed layer is significantly reduced allowing for much higher optical brightener levels to be used to optimize image quality. Locating the optical brightener in the layer adjacent to the exposed layer allows for a less expensive optical brightener to be used as the exposed layer, which is substantially free of optical brightener, prevents significant migration of the optical brightener. Another preferred method to reduce unwanted optical brightener migration is to use polypropylene for the layer adjacent to the exposed surface. Since optical brightener is more soluble in polypropylene than polyethylene, the optical brightener is less likely to migrate from polypropylene.

A biaxially oriented sheet of this invention, which has a microvoided core, is preferred. The microvoided core adds opacity and whiteness to the imaging support further improving imaging quality. Combining the image quality advantages of a microvoided core with a material which absorbs ultraviolet energy and emits light in the visible spectrum allows for the unique optimization of image quality as the image support can have a tint when exposed to ultraviolet energy yet retain excellent whiteness when the image is viewed using lighting that does not contain high amounts of ultraviolet energy such as some types of indoor lighting. The preferred number of voids in the vertical direction at substantially every point is greater than six. The number of voids in the vertical direction is the number of polymer/gas interfaces present in the voided layer. The voided layer functions as an opaque layer because of the index of refraction changes between polymer/gas interfaces. Greater than six voids is preferred because at 4 voids or less, little improvement in the opacity of the film is observed and thus does not justify the added expense to void the biaxially oriented sheet of this invention.

The biaxially oriented top sheet may also contain pigments, which are known to improve the photographic responses such as whiteness or sharpness. Titanium dioxide is used in this invention to improve image sharpness. The  $TiO_2$  used may be either anatase or rutile type. In the case of optical properties, rutile is the preferred because of the unique particle size and geometry. Further, both anatase and rutile  $TiO_2$  may be blended to improve both whiteness and sharpness. Examples of  $TiO_2$  that are acceptable for a photographic system are Dupont Chemical Co. R101 rutile  $TiO_2$  and DuPont Chemical Co. R104 rutile  $TiO_2$ . Other pigments to improve photographic responses may also be used in this invention such as titanium dioxide, barium sulfate, clay, or calcium carbonate. The preferred amount of  $TiO_2$  added to the biaxially oriented sheet of this invention

is between 18% and 24% by weight. Below 12% TiO<sub>2</sub>, the required reflection density of the biaxially oriented sheet is difficult to obtain. Above 28% TiO<sub>2</sub>, manufacturing efficiency declines because of problems extruding large amounts of TiO<sub>2</sub> compared with the base polymer. The hindered amine light stabilizer (HALS) may come from the common group of hindered amine compounds originating from 2,2,6,6-tetramethylpiperidine, and the term hindered amine light stabilizer is accepted to be used for hindered piperidine analogs. The compounds form stable nitroxyl radicals that interfere with photooxidation of polypropylene in the presence of oxygen, thereby affording excellent long-term photographic stability of the imaging element.

Because the display materials of the invention are subjected to changes in heat, humidity and UV radiation levels, HALS are used to stabilize the oriented polymer. The hindered amine will have sufficient molar mass to minimize migration in the final product, will be miscible with polypropylene at the preferred concentrations, and will not impart color to the final product. In the preferred embodiment, examples of HALS include poly{[6-[(1,1,3,3-tetramethylbutylamino)-1,3,5-triazine-4-piperidinyl]imino]-1,6-hexanediyl[(2,2,6,6-tetramethyl-4-piperidinyl)imino]} (Chimassorb 944 LD/FL), Chimassorb 119, and bis(1,2,2,6,6-pentamethyl-4-piperidinyl)[3,5-bis(1,1-dimethylethyl-4-hydroxyphenyl)methyl]butylpropanedioate (Timuvin 144), although they are not limited to these compounds.

In addition, the film may contain any of the hindered phenol primary antioxidants commonly used for thermal stabilization of polypropylene, alone, or in combination with secondary antioxidants. Examples of hindered phenol primary antioxidants include pentaerythritol tetrakis[3-(3,5-di-tert-butyl-4-hydroxyphenyl)propionate] (such as Irganox 1010), octadecyl 3-(3,5-di-tert-butyl-4-hydroxyphenyl)propionate (such as Irganox 1076), benzenepropanoic acid 3,5-bis(1,1-dimethyl)-4-hydroxy-2[3-[3,5-bis(1,1-dimethylethyl)-4-hydroxyphenyl]-1-oxopropyl]hydrazide (such as Irganox MD1024), 2,2'-thiodiethylenebis[3-(3,5-di-tert-butyl-4-hydroxyphenyl)propionate] (such as Irganox 1035), 1,3,5-trimethyl-2,4,6-tri(3,5-di-tert-butyl-4-hydroxybenzyl)-benzene (such as Irganox 1330), but are not limited to these examples. Secondary antioxidants include organic alkyl and aryl phosphites including examples such as triphenylphosphite (such as Irgastab TPP), tri(n-propylphenyl-phosphite) (such as Irgastab SN-55), 2,4-bis(1,1-dimethylphenyl)phosphite (such as Irgafos 168), and in a preferred embodiment would include Irgafos 168. The combination of hindered amines with other primary and secondary antioxidants have a synergistic benefit in a multilayer biaxially oriented polymer sheet by providing thermal stability to polymers such as polypropylene during melt processing and extrusion, and further enhancing their light and dark keeping properties which is not evident in a mono layer system for imaging products such as photographs. These unexpected results provide for a broader range of polymers that can be utilized in imaging product, thus enabling enhanced features to be incorporated into their design.

The preferred spectral transmission of the biaxially oriented top polyolefin sheet of this invention is less than 15%. Spectral transmission is the amount of light energy that is transmitted through a material. For a photographic element, spectral transmission is the ratio of the transmitted power to the incident power and is expressed as a percentage as follows;  $T_{RGB}=10^{-D}*100$  where D is the average of the red, green and blue Status A transmission density response measured by an X-Rite model 310 (or comparable) photo-

graphic transmission densitometer. The higher the transmission, the less opaque the material. For a reflective display material, the quality of the image is related to the amount of light reflected from the image to the observer's eye. A reflective image with a high amount of spectral transmission does not allow sufficient light to reach the observer's eye causing a perceptual loss in image quality. A reflective image with a spectral transmission of greater than 20% is unacceptable for a reflective display material as the quality of the image can not match prior art reflective display materials.

A reflection density of greater than 85% for the biaxially oriented sheet of this invention is preferred. Reflection density is the amount of light energy reflecting from the image to an observer's eye. Reflection density is measured by 0°/45° geometry Status A red/green/blue response using an X-Rite model 310 (or comparable) photographic transmission densitometer. A sufficient amount of reflective light energy is required to give the perception of image quality. A reflection density less than 75% is unacceptable for a reflective display material and does not match the quality of prior art reflective display materials.

Because the support materials of the invention are superior to prior art photographic base materials, the support materials utilized in this invention also are superior base materials for digital imaging technology other than silver halide products. By coating digital printing ink or dye receiver layers on the top of the support materials utilized in the invention, image quality and image durability can be improved over prior art materials. Examples of suitable digital imaging ink or dye receiver layer technology include ink jet printing receiver layers, thermal dye transfer receiving layers, and electrophotographic receiving layers. A preferred embodiment a reflection display material comprises an image, a laminated base material, and a scratch resistant polymer sheet laminated onto the top surface of said image. The laminated base material comprises an upper and lower biaxially oriented polymer sheet separated by a paper sheet, wherein said laminated base material has a thickness of greater than 254 micrometers, a stiffness of greater than 325 millinewtons in any direction, and an upper surface roughness of less than 0.45 micrometers at a spatial frequency of between 0.30 and 6.35 millimeters, and a transmission percent of less than 15 percent.

Said reflection display material in a much preferred form may be provided with a scratch resistant polymer sheet overlaying the image layer. Any suitable polymer sheet may be used such as polyester, polyolefin, or polyamide. In the most preferred embodiment the sheet comprises polycarbonate which may be further provided with a textured surface. Polycarbonate is highly desirable because it is a tough polymer sheet and offers superior scratch resistance. The scratch resistant polymer sheet has a scratch resistance of greater than 3 grams. This is preferred because it offers a wide range in scratch resistance and improved durability of prior practices. A resistant and stiff overlaying polycarbonate sheet is much preferred. Such a sheet is a suitable tough poster material. It may be rolled for storage and transported in a tube. The polycarbonate overcoated product is too stiff to process in conventional machinery, but as it is added after development, this is not a problem.

The coextrusion, quenching, orienting, and heat setting of these composite sheets may be effected by any process which is known in the art for producing oriented sheet, such as by a flat sheet process or a bubble or tubular process. The flat sheet process involves extruding the blend through a slit die and rapidly quenching the extruded web upon a chilled

casting drum so that the core matrix polymer component of the sheet and the skin components(s) are quenched below their glass solidification temperature. The quenched sheet is then biaxially oriented by stretching in mutually perpendicular directions at a temperature above the glass transition temperature, below the melting temperature of the matrix polymers. The sheet may be stretched in one direction and then in a second direction or may be simultaneously stretched in both directions. A stretching ratio defined as the final length divided by the original length for sum of the machine and cross directions, of at least 10 to 1 is preferred. After the sheet has been stretched, it is heat set by heating to a temperature sufficient to crystallize or anneal the polymers while restraining to some degree the sheet against retraction in both directions of stretching.

The top composite sheet, while described as having preferably at least three layers of a core and a skin layer on each side, may also be provided with additional layers that may serve to change the properties of the biaxially oriented sheet. Biaxially oriented sheets could be formed with surface layers that would provide an improved adhesion, or look to the support and photographic element. The biaxially oriented extrusion could be carried out with as many as 10 layers if desired to achieve some particular desired property.

These top and bottom composite sheets may be coated or treated after the coextrusion and orienting process or between casting and full orientation with any number of coatings which may be used to improve the properties of the sheets including printability, to provide a vapor barrier, to make them heat sealable, or to improve the adhesion to the support or to the photo sensitive layers. Examples of this would be acrylic coatings for printability, coating polyvinylidene chloride for heat seal properties. Further examples include flame, plasma or corona discharge treatment to improve printability or adhesion.

By having at least one nonvoided skin on the microvoided core, the tensile strength of the sheet is increased and makes it more manufacturable. It allows the sheets to be made at wider widths and higher draw ratios than when sheets are made with all layers voided. Coextruding the layers further simplifies the manufacturing process. In addition to a voided layer and a layer comprising  $TiO_2$ , the upper surface layer of the topside biaxially oriented sheet further comprises polyethylene. Polyethylene is preferred because it has superior adhesion to the gelatin in the photographic emulsions. In an additional embodiment the bottommost layer of the top biaxially oriented sheet comprises polyethylene or an ethylene copolymer. In such a case the adhesive layer used to adhere the biaxially oriented sheet to the paper base sheet may be a low density polyethylene. This has some cost advantages in that low density polyethylene is cheaper than a metallocene low density polyethylene.

The structure of a preferred display support where the imaging layers are applied to the biaxially oriented polyolefin sheet is as follows:

Biaxially oriented, microvoided polymer sheet With a top skin of polyethylene next to the image layer  
 High melt index polyethylene {>12 Melt Index (MI)}  
 Paper Base (>200 micrometers)  
 High melt index polyethylene {>12 Melt Index (MI)}  
 Biaxially oriented matte film  
 Conductive Layer

The support to which the microvoided composite sheets and biaxially oriented sheets are laminated for the laminated support of the photosensitive silver halide layer may be any paper sheet material with the desired refection, transmission

and stiffness properties. Photographic elements of the invention can be prepared on any suitable photographic paper support with a minimum paper thickness of 254 micrometers including synthetic paper and cellulose fiber paper.

5 Polyester sheets may be advantageous as the support because they provide excellent strength and dimensional stability. Such polyester sheets are well known, widely used and typically prepared from high molecular weight polyesters prepared by condensing a dihydric alcohol with a  
 10 dibasic saturated fatty acid or derivative thereof.

Suitable dihydric alcohols for use in preparing such polyesters are well known in the art and include any glycol wherein the hydroxyl groups are on the terminal carbon atom and contain from two to twelve carbon atoms such as,

15 for example, ethylene glycol, propylene glycol, trimethylene glycol, hexamethylene glycol, decamethylene glycol, dodecamethylene glycol, 1,4-cyclohexane, dimethanol, and the like.

Suitable dibasic acids useful for the preparation of polyesters include those containing from two to sixteen carbon atoms such as adipic acid, sebacic acid, isophthalic acid, terephthalic acid, and the like. Alkyl esters of acids such as those listed above can also be employed. Other alcohols and acids as well as polyesters prepared therefrom and the  
 20 preparation of the polyesters are described in U.S. Pat. Nos. 2,720,503 and 2,901,466. Polyethylene terephthalate is preferred.

Generally polyester film supports are prepared by melt extruding the polyester through a slit die, quenching to the amorphous state, orienting by machine and cross direction stretching and heat setting under dimensional restraint. The polyester film can also be subjected to a heat relaxation treatment to improve dimensional stability and surface smoothness.

35 The polyester film will typically contain an undercoat or primer layer on both sides of the polyester film. Subbing layers used to promote adhesion of coating compositions to the support are well known in the art and any such material can be employed. Some useful compositions for this purpose 40 include interpolymers of vinylidene chloride such as vinylidene chloride/methyl acrylate/itaconic acid terpolymers or vinylidene chloride/acrylonitrile/acrylic acid terpolymers, and the like. These and other suitable compositions are described, for example, in U.S. Pat. Nos. 2,627, 45 088; 2,698,240; 2,943,937; 3,143,421; 3,201,249; 3,271, 178; 3,443,950; 3,501,301 and the like. The polymeric subbing layer is usually overcoated with a second subbing layer comprised of gelatin, typically referred to as gel sub.

The base also may be a microvoided polyethylene 50 terephthalate such as disclosed in U.S. Pat. Nos. 4,912,333; 4,994,312 and 5,055,371.

When using a paper base, it is preferable to extrusion laminate the microvoided composite sheets to the base polymer using a polyolefin resin. Extrusion laminating is 55 carried out by bringing together the biaxially oriented sheets of the invention and the base sheet with application of an melt extruded adhesive between the base sheet and the biaxially oriented polyolefin sheets followed by their being pressed in a nip such as between two rollers. The melt- 60 extruded adhesive may be applied to either the biaxially oriented sheets or the base polymer prior to their being brought into the nip. In a preferred form the adhesive is applied into the nip simultaneously with the biaxially oriented sheets and the base polymer. The adhesive used to adhere the biaxially oriented polyolefin sheet to the polyester base may be any suitable material that does not have a harmful effect upon the photographic element. A preferred

material is metallocene catalyzed ethylene plastomers that are melt extruded into the nip between the polymer and the biaxially oriented sheet. Metallocene catalyzed ethylene plastomers are preferred because they are easily melt extruded, adhere well to biaxially oriented polyolefin sheets of this invention, and adhere well to gelatin sub coated polyester support of this invention. Another preferred melt adhesive is ethyl methyl acrylate or even a high melt index polyolefin such as polyethylene.

The preferred photographic element of this embodiment has a stiffness greater than 325 millinewtons and a thickness of greater than 254 micrometers and a surface roughness of less than 0.45 micrometers at a spatial frequency of between 0.30 and 6.35 millimeters and a transmission percent of 15 percent. At stiffness less than 325 millinewtons, the support becomes more difficult to convey through photoprocessing machines. The thickness of greater than 254 micrometers is preferred because it adds significant substance to the feel of the photographic display material. The most preferred embodiment of this invention has a paper sheet thickness of between 170 and 224 millimeters. Since this material is displayed with an image and often text, it is important to have a photographic element that has an exposure range of at least 125 nanoseconds to 0.5 seconds. Such a light sensitive photographic emulsion provides great digital compatibility such that both text and image can be exposed and developed without image flare. Very high D-max and D-mins are achieved. Furthermore it is important for said photographic element to have excellent smoothness and opacity. The preferred photographic element of this embodiment has a surface roughness of less than 0.45 micrometers at a spatial frequency of between 0.30 and 6.35 millimeters to minimize orange peel and a transmission percent of less than 15 percent to assure an adequate level of opacity to minimize show through. When paper base is used in the preferred embodiment, it is desirable to have a basis weight of greater than 200 g/m<sup>2</sup> to assure good handling and optical properties. The desired stiffness range of the photographic element of this invention is between 325 and 650 millinewtons. Below 325 millinewtons, it becomes more difficult to convey, and the base may have a tendency to crease when over laminating with a protective film. Elements with higher stiffness 500 to 650 millinewtons are desirable because they are more self-supporting when hung, and in most cases the very expensive overlaminates can be reduced in thickness resulting in a significant cost savings. Since the photographic element for display are often made on very thick pigmented polyester sheet, the photofinisher is accustomed to a highly reflective and very smooth base sheet. When forming a low cost element with biaxially oriented sheets and a paper base, it may be necessary to use very smooth paper. In the preferred embodiment the photographic element should have an upper surface roughness of between 0.20 and 0.50 micrometers. While roughness below 0.20 are obtainable, there are points of diminishing returns of achieving smoothness below 0.20, and when the roughness is above 0.50, there is also limited use. Roughness parameters are measured with a stylus type perthrometer that enables a two-dimensional tracing of the surface. The stylus is traversed normal to the surface at a constant speed. Results stated are mean values of several sampling lengths as stated in DIN 4762, ISO 4287/1 and 4288.

In order to have sufficient adhesion between the paper sheet and the biaxially oriented sheets, an adhesive layer is used to adhere the upper and lower biaxially oriented sheets to the paper base sheet. The adhesive material of this invention may be either a melt extrudable polymer such as

polyolefin, polyester, polyamide or polycarbonate or their copolymer derivatives or a room temperature adhesive. Selection of the specific type is largely dependent on base substrate and the biaxially oriented polymer sheet.

5 The preferred photographic element of this invention after the image has been fully formed and developed is then made into a superior reflection display material by overlaminating the photographic element with a scratch resistant polymer sheet onto the top surface of the image. In a preferred embodiment the scratch resistant polymer sheet is a polycarbonate sheet. While other overlaminates such as polyolefin, polyesters, and polyamides may be used when a superior scratch resistant overlaminated polymer sheet is desired, polycarbonate is the choice. Furthermore, a thick 10 sheet of polycarbonate adds stiffness and superior feel to the product. When selecting a scratch resistant polymer sheet, it should have a scratch resistance of greater than 0.2 micrograms of force. The scratch test is performed in an instrument that applies a controlled load to the surface of the material being tested. A stylus is used to produce the actual scratch. The type of material and geometry of stylus are important when comparing scratch propensity between different materials. The material composition, physical roughness, and thickness are important factors to control. 15 Another means to add value and improve scratch resistance is to provide a textured surface on the scratch resistant sheet. A textured surface may be embossed into the sheet or applied to the surface of the polymer overlaminated prior to its application to the photographic element or after it has 20 been overlaminated. To minimize scratches, fingerprinting and other issues, it is preferred to have a photographic element with an upper surface roughness of between 0.20 and 0.50 micrometers. A textured surface may also be achieved by two or more polymers being extruded as the 25 sheet or as a second layer if coextrusion is used to achieve a layer with roughness. In an additional embodiment of this invention, a coated layer on the overlaminated may be used to achieve the desired roughness. Typically a latex polymer is used as a binder in combination with an insoluble organic or inorganic particle such as methylacrylate bead or silica. Said scratch resistant polymer sheet with a textured surface 30 has a roughness average of 50 to 250 Ra.

35 A further embodiment of this invention provides a method of forming a reflection display material with a photographic element and at least one photosensitive layer. The base material of said invention comprises an upper and lower biaxially oriented polymer sheet and a base sheet, preferably paper, with a total thickness of at least 254 micrometers and a stiffness of 325 millinewtons in any direction with a upper 40 surface roughness of less than 0.45 micrometers at a spatial frequency of between 0.3 and 6.35 millimeters and a transmission percent of less than 15 percent. Said reflection display base material is formed with a developed and processed image that is brought into contact with a scratch 45 resistant polymer sheet. Furthermore, the scratch resistant polymer sheet is attached to the topmost layer of the final image by means of an adhesive. Said adhesive may be pre-coated on the scratch resistant polymer sheet or applied to either the polymer sheet or topmost layer of the image at 50 time of lamination. During lamination both the scratch resistant polymer sheet and the developed and processed imaged base material may be brought into contact with each other in a roller nip that applies pressure at room temperature or with application of heat to further enhance the bonding force among the materials.

55 As used herein, the phrase "photographic element" is a material that utilizes photosensitive silver halide in the

formation of images. The photographic elements can be black and white, single color elements or multicolor elements. Multicolor elements contain image dye-forming units sensitive to each of the three primary regions of the spectrum. Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

The photographic emulsions useful for this invention are generally prepared by precipitating silver halide crystals in a colloidal matrix by methods conventional in the art. The colloid is typically a hydrophilic film-forming agent such as gelatin, alginic acid, or derivatives thereof.

The crystals formed in the precipitation step are washed and then chemically and spectrally sensitized by adding spectral sensitizing dyes and chemical sensitizers, and by providing a heating step during which the emulsion temperature is raised, typically from 40° C. to 70° C., and maintained for a period of time. The precipitation and spectral and chemical sensitization methods utilized in preparing the emulsions employed in the invention can be those methods known in the art.

This invention is directed to a silver halide photographic element capable of excellent performance when exposed by either an electronic printing method or a conventional optical printing method. An electronic printing method comprises subjecting a radiation sensitive silver halide emulsion layer of a recording element to actinic radiation of at least  $10^{-4}$  ergs/cm<sup>2</sup> for up to 100 $\mu$  seconds duration in a pixel-by-pixel mode wherein the silver halide emulsion layer is comprised of silver halide grains as described above. A conventional optical printing method comprises subjecting a radiation sensitive silver halide emulsion layer of a recording element to actinic radiation of at least  $10^{-4}$  ergs/cm<sup>2</sup> for 10<sup>-3</sup> to 300 seconds in an imagewise mode wherein the silver halide emulsion layer is comprised of silver halide grains as described above.

This invention in a preferred embodiment utilizes a radiation-sensitive emulsion comprised of silver halide grains (a) containing greater than 50 mole percent chloride, based on silver, (b) having greater than 50 percent of their surface area provided by {100} crystal faces, and (c) having a central portion accounting for from 95 to 99 percent of total silver and containing two dopants selected to satisfy each of the following class requirements: (i) a hexacoordination metal complex which satisfies the formula



(I)

wherein n is zero, -1, -2, -3 or -4; M is a filled frontier orbital polyvalent metal ion, other than iridium; and L<sub>6</sub> represents bridging ligands which can be independently selected, provided that least four of the ligands are anionic ligands, and at least one of the ligands is a cyano ligand and (ii) an iridium coordination complex containing a thiazole or substituted thiazole ligand.

This invention is directed towards a photographic recording element comprising a support and at least one light sensitive silver halide emulsion layer comprising silver halide grains as described above.

It has been discovered quite surprisingly that the combination of dopants (i) and (ii) provides greater reduction in reciprocity law failure than can be achieved with either dopant alone. Further, unexpectedly, the combination of

dopants (i) and (ii) achieve reductions in reciprocity law failure beyond the simple additive sum achieved when employing either dopant class by itself. It has not been reported or suggested prior to this invention that the combination of dopants (i) and (ii) provides greater reduction in reciprocity law failure, particularly for high intensity and short duration exposures. The combination of dopants (i) and (ii) further unexpectedly achieves high intensity reciprocity with iridium at relatively low levels, and both high and low intensity reciprocity improvements even while using conventional gelatino-peptizer (e.g., other than low methionine gelatino-peptizer). Furthermore, unexpectedly, when the light sensitive emulsion of this invention is applied to a base material with an upper and lower biaxially oriented sheet with the upper biaxially oriented sheet comprising voids in at least one layer and white pigment in at least one layer and the layer comprising white pigment further comprises light and thermal stabilizing agents that a superior imaging material with long life as well as superior sharpness and compatibility with digital exposing devices.

In a preferred practical application, the advantages of the invention can be transformed into increased throughput of digital substantially artifact-free color print images while exposing each pixel sequentially in synchronism with the digital data from an image processor.

In one embodiment, the present invention represents an improvement on the electronic printing method. Specifically, this invention in one embodiment is directed to an electronic printing method which comprises subjecting a radiation sensitive silver halide emulsion layer of a recording element to actinic radiation of at least  $10^{-4}$  ergs/cm<sup>2</sup> for up to 100 $\mu$  seconds duration in a pixel-by-pixel mode. The present invention realizes an improvement in reciprocity failure by selection of the radiation sensitive silver halide emulsion layer. While certain embodiments of the invention are specifically directed towards electronic printing, use of the emulsions and elements of the invention is not limited to such specific embodiment, and it is specifically contemplated that the emulsions and elements of the invention are also well suited for conventional optical printing.

It has been found that significantly improved reciprocity performance can be obtained for silver halide grains (a) containing greater than 50 mole percent chloride, based on silver, and (b) having greater than 50 percent of their surface area provided by {100} crystal faces by employing a hexacoordination complex dopant of class (i) in combination with an iridium complex dopant comprising a thiazole or substituted thiazole ligand. The reciprocity improvement is obtained for silver halide grains employing conventional gelatino-peptizer, unlike the contrast improvement described for the combination of dopants set forth in U.S. Pat. Nos. 5,783,373 and 5,783,378, which requires the use of low methionine gelatino-peptizers as discussed therein, and which states it is preferable to limit the concentration of any gelatino-peptizer with a methionine level of greater than 30 micromoles per gram to a concentration of less than 1 percent of the total peptizer employed. Accordingly, in specific embodiments of the invention, it is specifically contemplated to use significant levels (i.e., greater than 1 weight percent of total peptizer) of conventional gelatin (e.g., gelatin having at least 30 micromoles of methionine per gram) as a gelatino-peptizer for the silver halide grains of the emulsions of the invention. In preferred embodiments of the invention, gelatino-peptizer is employed which comprises at least 50 weight percent of gelatin containing at least 30 micromoles of methionine per gram, as it is frequently desirable to limit the level of oxidized low methionine gelatin which may be used for cost and certain performance reasons.

In a specific, preferred form of the invention it is contemplated to employ a class (i) hexacoordination complex dopant satisfying the formula:



where

$n$  is zero, -1, -2, -3 or -4;

M is a filled frontier orbital polyvalent metal ion, other than iridium, preferably  $Fe^{+2}$ ,  $Ru^{+2}$ ,  $Os^{+2}$ ,  $Co^{+3}$ ,  $Rh^{+3}$ ,  $Pd^{+4}$  or  $Pt^{+4}$ , more preferably an iron, ruthenium or osmium ion, and most preferably a ruthenium ion;

$L_6$  represents six bridging ligands which can be independently selected, provided that least four of the ligands are anionic ligands and at least one (preferably at least 3 and optimally at least 4) of the ligands is a cyano ligand or a ligand more electronegative than a cyano ligand. Any remaining ligands can be selected from among various other bridging ligands, including aquo ligands, halide ligands (specifically, fluoride, chloride, bromide and iodide), cyanate ligands, thiocyanate ligands, selenocyanate ligands, tellurocyanate ligands, and azide ligands. Hexacoordinated transition metal complexes of class (i) which include six cyano ligands are specifically preferred.

Illustrations of specifically contemplated class (i) hexacoordination complexes for inclusion in the high chloride grains are provided by Olm et al U.S. Pat. No. 5,503,970 and Daubendiek et al U.S. Pat. Nos. 5,494,789 and 5,503,971, and Keevert et al U.S. Pat. No. 4,945,035, as well as Murakami et al Japanese Patent Application Hei-2[1990]-249588, and *Research Disclosure* Item 36736. Useful neutral and anionic organic ligands for class (ii) dopant hexacoordination complexes are disclosed by Olm et al U.S. Pat. No. 5,360,712 and Kuromoto et al U.S. Pat. No. 5,462,849.

Class (i) dopant is preferably introduced into the high chloride grains after at least 50 (most preferably 75 and optimally 80) percent of the silver has been precipitated, but before precipitation of the central portion of the grains has been completed. Preferably class (i) dopant is introduced before 98 (most preferably 95 and optimally 90) percent of the silver has been precipitated. Stated in terms of the fully precipitated grain structure, class (i) dopant is preferably present in an interior shell region that surrounds at least 50 (most preferably 75 and optimally 80) percent of the silver and, with the more centrally located silver, accounts the entire central portion (99 percent of the silver), most preferably accounts for 95 percent, and optimally accounts for 90 percent of the silver halide forming the high chloride grains. The class (i) dopant can be distributed throughout the interior shell region delimited above or can be added as one or more bands within the interior shell region.

Class (i) dopant can be employed in any conventional useful concentration. A preferred concentration range is from  $10^{-8}$  to  $10^{-3}$  mole per silver mole, most preferably from  $10^{-6}$  to  $5 \times 10^{-4}$  mole per silver mole.

The following are specific illustrations of class (i) dopants:

- (i-1)  $[Fe(CN)_6]^{-4}$
- (i-2)  $[Ru(CN)_6]^{-4}$
- (i-3)  $[Os(CN)_6]^{-4}$
- (i-4)  $[Rh(CN)_6]^{-3}$
- (i-5)  $[Co(CN)_6]^{-3}$
- (i-6)  $[Fe(pyrazine)(CN)_5]^{-4}$
- (i-7)  $[RuCl(CN)_5]^{-4}$
- (i-8)  $[OsBr(CN)_5]^{-4}$
- (i-9)  $[RhF(CN)_5]^{-3}$

- (i-10)  $[In(NCS)_6]^{-3}$
- (i-11)  $[FeCO(CN)_5]^{-3}$
- (i-12)  $[RuF_2(CN)_4]^{-4}$
- (i-13)  $[OsCl_2(CN)_4]^{-4}$
- (i-14)  $[RhI_2(CN)_4]^{-3}$
- (i-15)  $[Ga(NCS)_6]^{-3}$
- (i-16)  $[Ru(CN)_5(OCN)]^{-4}$
- (i-17)  $[Ru(CN)_5(N_3)]^{-4}$
- (i-18)  $[Os(CN)_5(SCN)]^{-4}$
- (i-19)  $[Rh(CN)_5(SeCN)]^{-3}$
- (i-20)  $[Os(CN)Cl_5]^{-4}$
- (i-21)  $[Fe(CN)_3Cl_3]^{-3}$
- (i-22)  $[Ru(CO)_2(CN)_4]^{-1}$

When the class (i) dopants have a net negative charge, it is appreciated that they are associated with a counter ion when added to the reaction vessel during precipitation. The counter ion is of little importance, since it is ionically dissociated from the dopant in solution and is not incorporated within the grain. Common counter ions known to be fully compatible with silver chloride precipitation, such as ammonium and alkali metal ions, are contemplated. It is noted that the same comments apply to class (ii) dopants, otherwise described below.

The class (ii) dopant is an iridium coordination complex containing at least one thiazole or substituted thiazole ligand. Careful scientific investigations have revealed Group VIII hexahalo coordination complexes to create deep electron traps, as illustrated R. S. Eachus, R. E. Graves and M. T. Olm *J. Chem. Phys.*, Vol. 69, pp. 4580-7 (1978) and *Physica Status Solidi A*, Vol. 57, 429-37 (1980) and R. S. Eachus and M. T. Olm *Annu. Rep. Prog. Chem. Sect. C. Phys. Chem.*, Vol. 83, 3, pp. 3-48 (1986). The class (ii) dopants employed in the practice of this invention are believed to create such deep electron traps. The thiazole ligands may be substituted with any photographically acceptable substituent which does not prevent incorporation of the dopant into the silver halide grain. Exemplary substituents include lower alkyl (e.g., alkyl groups containing 1-4 carbon atoms), and specifically methyl. A specific example of a substituted thiazole ligand which may be used in accordance with the invention is 5-methylthiazole. The class (ii) dopant preferably is an iridium coordination complex having ligands each of which are more electropositive than a cyano ligand. In a specifically preferred form the remaining non-thiazole or non-substituted-thiazole ligands of the coordination complexes forming class (ii) dopants are halide ligands.

It is specifically contemplated to select class (ii) dopants from among the coordination complexes containing organic ligands disclosed by Olm et al U.S. Pat. No. 5,360,712, Olm et al U.S. Pat. No. 5,457,021 and Kuromoto et al U.S. Pat. No. 5,462,849.

In a preferred form it is contemplated to employ as a class (ii) dopant a hexacoordination complex satisfying the formula:



wherein

$n'$  is zero, -1, -2, -3 or -4; and

60  $L_6$  represents six bridging ligands which can be independently selected, provided that at least four of the ligands are anionic ligands, each of the ligands is more electropositive than a cyano ligand, and at least one of the ligands comprises a thiazole or substituted thiazole ligand. In a specifically preferred form at least four of the ligands are halide ligands, such as chloride or bromide ligands.

Class (ii) dopant is preferably introduced into the high chloride grains after at least 50 (most preferably 85 and optimally 90) percent of the silver has been precipitated, but before precipitation of the central portion of the grains has been completed. Preferably class (ii) dopant is introduced before 99 (most preferably 97 and optimally 95) percent of the silver has been precipitated. Stated in terms of the fully precipitated grain structure, class (ii) dopant is preferably present in an interior shell region that surrounds at least 50 (most preferably 85 and optimally 90) percent of the silver and, with the more centrally located silver, accounts the entire central portion (99 percent of the silver), most preferably accounts for 97 percent, and optimally accounts for 95 percent of the silver halide forming the high chloride grains. The class (ii) dopant can be distributed throughout the interior shell region delimited above or can be added as one or more bands within the interior shell region.

Class (ii) dopant can be employed in any conventional useful concentration. A preferred concentration range is from  $10^{-9}$  to  $10^{-4}$  mole per silver mole. Iridium is most preferably employed in a concentration range of from  $10^{-8}$  to  $10^{-5}$  mole per silver mole.

Specific illustrations of class (ii) dopants are the following:

- (ii-1)  $[\text{IrCl}_5(\text{thiazole})]^{2-}$
- (ii-2)  $[\text{IrCl}_4(\text{thiazole})_2]^{-1}$
- (ii-3)  $[\text{IrBr}_5(\text{thiazole})]^{2-}$
- (ii-4)  $[\text{IrBr}_4(\text{thiazole})_2]^{-1}$
- (ii-5)  $[\text{IrCl}_5(5\text{-methylthiazole})]^{2-}$
- (ii-6)  $[\text{IrCl}_4(5\text{-methylthiazole})_2]^{-1}$
- (ii-7)  $[\text{IrBr}_5(5\text{-methylthiazole})]^{2-}$
- (ii-8)  $[\text{IrBr}_4(5\text{-methylthiazole})_2]^{-1}$

In one preferred aspect of the invention in a layer using a magenta dye forming coupler, a class (ii) dopant in combination with an  $\text{OsCl}_5(\text{NO})$  dopant has been found to produce a preferred result.

Emulsions demonstrating the advantages of the invention can be realized by modifying the precipitation of conventional high chloride silver halide grains having predominantly (>50%) {100} crystal faces by employing a combination of class (i) and (ii) dopants as described above.

The silver halide grains precipitated contain greater than 50 mole percent chloride, based on silver. Preferably the grains contain at least 70 mole percent chloride and, optimally at least 90 mole percent chloride, based on silver. Iodide can be present in the grains up to its solubility limit, which is in silver iodochloride grains, under typical conditions of precipitation, about 11 mole percent, based on silver. It is preferred for most photographic applications to limit iodide to less than 5 mole percent iodide, most preferably less than 2 mole percent iodide, based on silver.

Silver bromide and silver chloride are miscible in all proportions. Hence, any portion, up to 50 mole percent, of the total halide not accounted for chloride and iodide, can be bromide. For color reflection print (i.e., color paper) uses bromide is typically limited to less than 10 mole percent based on silver and iodide is limited to less than 1 mole percent based on silver.

In a widely used form high chloride grains are precipitated to form cubic grains--that is, grains having {100} major faces and edges of equal length. In practice ripening effects usually round the edges and corners of the grains to some extent. However, except under extreme ripening conditions substantially more than 50 percent of total grain surface area is accounted for by {100} crystal faces.

High chloride tetradecahedral grains are a common variant of cubic grains. These grains contain 6 {100} crystal

faces and 8 {111} crystal faces. Tetradecahedral grains are within the contemplation of this invention to the extent that greater than 50 percent of total surface area is accounted for by {100} crystal faces.

Although it is common practice to avoid or minimize the incorporation of iodide into high chloride grains employed in color paper, it is has been recently observed that silver iodochloride grains with {100} crystal faces and, in some instances, one or more {111} faces offer exceptional levels of photographic speed. In these emulsions iodide is incorporated in overall concentrations of from 0.05 to 3.0 mole percent, based on silver, with the grains having a surface shell of greater than 50 Å that is substantially free of iodide and a interior shell having a maximum iodide concentration that surrounds a core accounting for at least 50 percent of total silver. Such grain structures are illustrated by Chen et al EPO 0 718 679.

In another improved form the high chloride grains can take the form of tabular grains having {100} major faces. Preferred high chloride {100} tabular grain emulsions are those in which the tabular grains account for at least 70 (most preferably at least 90) percent of total grain projected area. Preferred high chloride {100} tabular grain emulsions have average aspect ratios of at least 5 (most preferably at least >8). Tabular grains typically have thicknesses of less than 0.3  $\mu\text{m}$ , preferably less than 0.2  $\mu\text{m}$ , and optimally less than 0.07  $\mu\text{m}$ . High chloride {100} tabular grain emulsions and their preparation are disclosed by Maskasky U.S. Pat. Nos. 5,264,337 and 5,292,632; House et al U.S. Pat. No. 5,320,938; Brust et al U.S. Pat. No. 5,314,798; and Chang et al U.S. Pat. No. 5,413,904.

Once high chloride grains having predominantly {100} crystal faces have been precipitated with a combination of class (i) and class (ii) dopants described above, chemical and spectral sensitization, followed by the addition of conventional addenda to adapt the emulsion for the imaging application of choice can take any convenient conventional form. These conventional features are illustrated by *Research Disclosure*, Item 38957, cited above, particularly:

- III. Emulsion washing;
- IV. Chemical sensitization;
- V. Spectral sensitization and desensitization;
- VII. Antifoggants and stabilizers;
- VIII. Absorbing and scattering materials;
- IX. Coating and physical property modifying addenda; and
- X. Dye image formers and modifiers.

Some additional silver halide, typically less than 1 percent, based on total silver, can be introduced to facilitate chemical sensitization. It is also recognized that silver halide can be epitaxially deposited at selected sites on a host grain to increase its sensitivity. For example, high chloride {100} tabular grains with corner epitaxy are illustrated by Maskasky U.S. Pat. No. 5,275,930. For the purpose of providing a clear demarcation, the term "silver halide grain" is herein employed to include the silver necessary to form the grain up to the point that the final {100} crystal faces of the grain are formed. Silver halide later deposited that does not overlie the {100} crystal faces previously formed accounting for at least 50 percent of the grain surface area is excluded in determining total silver forming the silver halide grains. Thus, the silver forming selected site epitaxy is not part of the silver halide grains while silver halide that deposits and provides the final {100} crystal faces of the grains is included in the total silver forming the grains, even when it differs significantly in composition from the previously precipitated silver halide.

The emulsions can be spectrally sensitized with any of the dyes known to the photographic art, such as the polymethine

**21**

dye class, which includes the cyanines, merocyanines, complex cyanines and merocyanines, oxonols, hemioxonols, styryls, merostyryls and streptocyanines. In particular, it would be advantageous to select from among the low staining sensitizing dyes disclosed in U.S. Pat. Nos. 5,292,634; 5,316,904; 5,418,126 and 5,492,802. Use of low staining sensitizing dyes in a photographic element processed in a developer solution with little or no optical brightening agent (for instance, stilbene compounds such as Blankophor REU™) is specifically contemplated. Further, these low staining dyes can be used in combination with other dyes known to the art (*Research Disclosure*, September 1996, Item 38957, Section V).

Useful sensitizing dyes include, but are not limited to, the following.



BSD-1

20

25

30

40

BSD-3

45

50

55

60

**22**

-continued

GSD-1



GSD-2



GSD-3



GSD-4



-continued



Emulsions can be spectrally sensitized with mixtures of two or more sensitizing dyes which form mixed dye aggregates on the surface of the emulsion grain. The use of mixed dye aggregates enables adjustment of the spectral sensitivity of the emulsion to any wavelength between the extremes of the wavelengths of peak sensitivities ( $\lambda$ -max) of the two or more dyes. This practice is especially valuable if the two or more sensitizing dyes absorb in similar portions of the spectrum (i.e., blue, or green or red and not green plus red or blue plus red or green plus blue). Since the function of the spectral sensitizing dye is to modulate the information recorded in the negative which is recorded as an image dye, positioning the peak spectral sensitivity at or near the  $\lambda$ -max of the image dye in the color negative produces the optimum preferred response. In addition, the combination of similarly spectrally sensitized emulsions can be in one or more layers.

An important quality characteristic of a reproductive film system is color reproduction, which represents how accurately the hues of the original scene are reproduced. Many current color papers use a blue sensitizing dye that gives a maximum sensitivity at about 480 nm. Use of a sensitizing dye that affords a sensitivity maximum that is closer to that of the yellow image dye in film, for instance with a sensitivity maximum of around 450–470 nm, can result in a color paper with improved color reproduction.

In the simplest contemplated form a recording element contemplated for use in the electronic printing method of one embodiment of the invention can consist of a single emulsion layer satisfying the emulsion description provided above coated on a conventional photographic support, such

as those described in *Research Disclosure*, Item 38957, cited above, XVI. Supports. In one preferred form the support is a white reflective support, such as photographic paper support or a film support that contains or bears a coating of a reflective pigment. To permit a print image to be viewed using an illuminant placed behind the support, it is preferred to employ a white translucent support, such as a Duratrans<sup>TM</sup> or Duraclear<sup>TM</sup> support.

Image dye-forming couplers may be included in the element such as couplers that form cyan dyes upon reaction with oxidized color developing agents which are described in such representative patents and publications as: U.S. Pat. Nos. 2,367,531; 2,423,730; 2,474,293; 2,772,162; 2,895,826; 3,002,836; 3,034,892; 3,041,236; 4,883,746 and 15 “Farbkuppler—Eine Literature Übersicht,” published in Agfa Mitteilungen, Band III, pp. 156–175 (1961). Preferably such couplers are phenols and naphthols that form cyan dyes on reaction with oxidized color developing agent. Also preferable are the cyan couplers described in, for instance, European Patent Application Nos. 491,197; 544,322; 556,700; 556,777; 565,096; 570,006; and 574,948.

Typical cyan couplers are represented by the following formulas:

CYAN-1



CYAN-2



CYAN-3



CYAN-4



wherein R<sub>1</sub>, R<sub>5</sub> and R<sub>8</sub> each represents a hydrogen or a substituent; R<sub>2</sub> represents a substituent; R<sub>3</sub>, R<sub>4</sub> and R<sub>7</sub> each represent an electron attractive group having a Hammett's substituent constant  $\sigma_{para}$  of 0.2 or more and the sum of the  $\sigma_{para}$  values of R<sub>3</sub> and R<sub>4</sub> is 0.65 or more; R<sub>6</sub> represents an electron attractive group having a Hammett's substituent constant  $\sigma_{para}$  of 0.35 or more; X represents a hydrogen or a coupling-off group; Z<sub>1</sub> represents nonmetallic atoms necessary for forming a nitrogen-containing, six-membered, heterocyclic ring which has at least one dissociative group; Z<sub>2</sub> represents  $-\text{C}(\text{R}_7)=$  and  $-\text{N}=\text{}$ ; and Z<sub>3</sub> and Z<sub>4</sub> each represents  $-\text{C}(\text{R}_8)=$  and  $-\text{N}=\text{}$ .

For purposes of this invention, an “NB coupler” is a dye-forming coupler which is capable of coupling with the developer 4-amino-3-methyl-N-ethyl-N-(2-methanesulfonamidoethyl)aniline sesquisulfate hydrate to

form a dye for which the left bandwidth (LBW) of its absorption spectra upon "spin coating" of a 3% w/v solution of the dye in di-n-butyl sebacate solvent is at least 5 nm. less than the LBW for a 3% w/v solution of the same dye in acetonitrile. The LBW of the spectral curve for a dye is the distance between the left side of the spectral curve and the wavelength of maximum absorption measured at a density of half the maximum.

The "spin coating" sample is prepared by first preparing a solution of the dye in di-n-butyl sebacate solvent (3% w/v). If the dye is insoluble, dissolution is achieved by the addition of some methylene chloride. The solution is filtered and 0.1-0.2 ml is applied to a clear polyethylene terephthalate support (approximately 4 cm×4 cm) and spun at 4,000 RPM using the Spin Coating equipment, Model No. EC101, available from Headway Research Inc., Garland, Tex. The transmission spectra of the so prepared dye samples are then recorded.

Preferred "NB couplers" form a dye which, in n-butyl sebacate, has a LBW of the absorption spectra upon "spin coating" which is at least 15 nm, preferably at least 25 nm, less than that of the same dye in a 3% solution (w/v) in acetonitrile.

In a preferred embodiment the cyan dye-forming "NB coupler" useful in the invention has the formula (IA)

(IA)



wherein

R' and R'' are substituents selected such that the coupler is a "NB coupler", as herein defined; and

Z is a hydrogen atom or a group which can be split off by the reaction of the coupler with an oxidized color developing agent.

The coupler of formula (IA) is a 2,5-diamido phenolic cyan coupler wherein the substituents R' and R'' are preferably independently selected from unsubstituted or substituted alkyl, aryl, amino, alkoxy and heterocyclyl groups.

In a further preferred embodiment, the "NB coupler" has the formula (I):

(I)



wherein

R'' and R''' are independently selected from unsubstituted or substituted alkyl, aryl, amino, alkoxy and heterocyclyl groups and Z is as hereinbefore defined;

R<sub>1</sub> and R<sub>2</sub> are independently hydrogen or an unsubstituted or substituted alkyl group.

Typically, R'' is an alkyl, amino or aryl group, suitably a phenyl group. R''' is desirably an alkyl or aryl group or a 5-10 membered heterocyclic ring which contains one or more heteroatoms selected from nitrogen, oxygen and sulfur, which ring group is unsubstituted or substituted.

In the preferred embodiment the coupler of formula (I) is a 2,5-diamido phenol in which the 5-amido moiety is an amide of a carboxylic acid which is substituted in the alpha position by a particular sulfone (—SO<sub>2</sub><sup>+</sup>) group, such as, for example, described in U.S. Pat. No. 5,686,235. The sulfone moiety is an unsubstituted or substituted alkylsulfone or a heterocyclic sulfone or it is an arylsulfone, which is preferably substituted, in particular in the meta and/or para position.

Couplers having these structures of formulae (I) or (IA) comprise cyan dye-forming "NB couplers" which form image dyes having very sharp-cutting dye hues on the short wavelength side of the absorption curves with absorption maxima ( $\lambda_{max}$ ) which are shifted hypsochromically and are generally in the range of 620-645 nm, which is ideally suited for producing excellent color reproduction and high color saturation in color photographic papers.

Referring to formula (I), R<sub>1</sub> and R<sub>2</sub> are independently hydrogen or an unsubstituted or substituted alkyl group, preferably having from 1 to 24 carbon atoms and in particular 1 to 10 carbon atoms, suitably a methyl, ethyl, n-propyl, isopropyl, butyl or decyl group or an alkyl group substituted with one or more fluoro, chloro or bromo atoms, such as a trifluoromethyl group. Suitably, at least one of R<sub>1</sub> and R<sub>2</sub> is a hydrogen atom and if only one of R<sub>1</sub> and R<sub>2</sub> is a hydrogen atom then the other is preferably an alkyl group having 1 to 4 carbon atoms, more preferably one to three carbon atoms and desirably two carbon atoms.

As used herein and throughout the specification unless where specifically stated otherwise, the term "alkyl" refers to an unsaturated or saturated straight or branched chain alkyl group, including alkenyl, and includes aralkyl and cyclic alkyl groups, including cycloalkenyl, having 3-8 carbon atoms and the term 'aryl' includes specifically fused aryl.

In formula (I), R'' is suitably an unsubstituted or substituted amino, alkyl or aryl group or a 5-10 membered heterocyclic ring which contains one or more heteroatoms selected from nitrogen, oxygen and sulfur, which ring is unsubstituted or substituted, but is more suitably an unsubstituted or substituted phenyl group.

Examples of suitable substituent groups for this aryl or heterocyclic ring include cyano, chloro, fluoro, bromo, iodo, alkyl- or aryl-carbonyl, alkyl- or aryl-oxycarbonyl, carbonamido, alkyl- or aryl-carbonamido, alkyl- or aryl-sulfonyl, alkyl- or aryl-sulfonyloxy, alkyl- or aryl-oxysulfonyl, alkyl- or aryl-sulfoxide, alkyl- or aryl-sulfamoyl, alkyl- or aryl-sulfonamido, aryl, alkyl, alkoxy, aryloxy, nitro, alkyl- or aryl-ureido and alkyl- or aryl-carbamoyl groups, any of which may be further substituted.

Preferred groups are halogen, cyano, alkoxy carbonyl, alkylsulfamoyl, alkyl-sulfonamido, alkylsulfonyl, carbamoyl, alkylcarbamoyl or alkylcarbonamido. Suitably, R'' is a 4-chlorophenyl, 3,4-di-chlorophenyl, 3,4-difluorophenyl, 4-cyanophenyl, 3-chloro-4-cyanophenyl, pentafluorophenyl, or a 3- or 4-sulfonamidophenyl group.

In formula (I), when R''' is alkyl, it may be unsubstituted or substituted with a substituent such as halogen or alkoxy. When R''' is aryl or a heterocycle, it may be substituted. Desirably it is not substituted in the position alpha to the sulfonyl group.

In formula (I), when R''' is a phenyl group, it may be substituted in the meta and/or para positions with one to

three substituents independently selected from the group consisting of halogen, and unsubstituted or substituted alkyl, alkoxy, aryloxy, acyloxy, acylamino, alkyl- or aryl-sulfonyloxy, alkyl- or aryl-sulfamoyl, alkyl- or aryl-sulfamoyl amino, alkyl- or aryl-sulfonamido, alkyl- or aryl-ureido, alkyl- or aryl-oxycarbonyl, alkyl- or aryl-oxy-carbonylamino and alkyl- or aryl-carbamoyl groups.

In particular each substituent may be an alkyl group such as methyl, t-butyl, heptyl, dodecyl, pentadecyl, octadecyl or 1,1,2,2-tetramethylpropyl; an alkoxy group such as methoxy, t-butoxy, octyloxy, dodecyloxy, tetradecyloxy, hexadecyloxy or octadecyloxy; an aryloxy group such as phenoxy, 4-t-butylphenoxy or 4-dodecyl-phenoxy; an alkyl- or aryl-acyloxy group such as acetoxy or dodecanoyloxy; an alkyl- or aryl-acylamino group such as acetamido, hexadecanamido or benzamido; an alkyl- or aryl-sulfonyloxy group such as methyl-sulfonyloxy, dodecylsulfonyloxy or 4-methylphenyl-sulfonyloxy; an alkyl- or aryl-sulfamoyl-group such as N-butylsulfamoyl or N-4-t-butylphenylsulfamoyl; an alkyl- or aryl-sulfamoylamino group such as N-butyl-sulfamoylamino or N-4-t-butylphenylsulfamoyl-amino; an alkyl- or aryl-sulfonamido group such as methane-sulfonamido, hexadecanesulfonamido or 4-chlorophenyl-sulfonamido; an alkyl- or arylureido group such as methylureido or phenylureido; an alkoxy- or aryloxy-carbonyl such as methoxycarbonyl or phenoxy carbonyl; an alkoxy- or aryloxy-carbonylamino group such as methoxy-carbonylamino or phenoxy carbonylamino; an alkyl- or aryl-carbamoyl group such as N-butylcarbamoyl or N-methyl-N-dodecylcarbamoyl; or a perfluoroalkyl group such as trifluoromethyl or heptafluoropropyl.

Suitably the above substituent groups have 1 to 30 carbon atoms, more preferably 8 to 20 aliphatic carbon atoms. A desirable substituent is an alkyl group of 12 to 18 aliphatic carbon atoms such as dodecyl, pentadecyl or octadecyl or an alkoxy group with 8 to 18 aliphatic carbon atoms such as dodecyloxy and hexadecyoxy or a halogen such as a meta or para chloro group, carboxy or sulfonamido. Any such groups may contain interrupting heteroatoms such as oxygen to form e.g. polyalkylene oxides.

In formula (I) or (IA) Z is a hydrogen atom or a group which can be split off by the reaction of the coupler with an oxidized color developing agent, known in the photographic art as a 'coupling-off group' and may preferably be 45 hydrogen, chloro, fluoro, substituted aryloxy or mercaptotetrazole, more preferably hydrogen or chloro.

The presence or absence of such groups determines the chemical equivalency of the coupler, i.e., whether it is a 2-equivalent or 4-equivalent coupler, and its particular identity can modify the reactivity of the coupler. Such groups can advantageously affect the layer in which the coupler is coated, or other layers in the photographic recording material, by performing, after release from the coupler, functions such as dye formation, dye hue adjustment, development acceleration or inhibition, bleach acceleration or inhibition, electron transfer facilitation, color correction, and the like.

Representative classes of such coupling-off groups include, for example, halogen, alkoxy, aryloxy, heterocyclxy, sulfonyloxy, acyloxy, acyl, heterocyclsulfonamido, heterocyclthio, benzothiazolyl, phosphonyloxy, alkylthio, arylthio, and arylazo. These coupling-off groups are described in the art, for example, in U.S. Pat. Nos. 2,455,169; 3,227,551; 3,432,521; 3,467,563; 3,617,291; 3,880,661; 4,052,212; and 4,134,766; and in U.K. Patent Nos. and published applications 1,466,728;

1,531,927; 1,533,039; 2,066,755A, and 2,017,704A. Halogen, alkoxy and aryloxy groups are most suitable.

Examples of specific coupling-off groups are  $-\text{Cl}$ ,  $-\text{F}$ ,  $-\text{Br}$ ,  $-\text{SCN}$ ,  $-\text{OCH}_3$ ,  $-\text{OC}_6\text{H}_5$ ,  $-\text{OCH}_2\text{C}(=\text{O})\text{NHCH}_2\text{CH}_2\text{OH}$ ,  $-\text{OCH}_2\text{C}(\text{O})\text{NHCH}_2\text{CH}_2\text{OCH}_3$ ,  $-\text{OCH}_2\text{C}(\text{O})\text{NHCH}_2\text{CH}_2\text{OC}(=\text{O})\text{OCH}_3$ ,  $-\text{P}(\text{O})(\text{OC}_2\text{H}_5)_2$ ,  $-\text{SCH}_2\text{CH}_2\text{COOH}$ ,



Typically, the coupling-off group is a chlorine atom, hydrogen atom or p-methoxyphenoxy group.

It is essential that the substituent groups be selected so as to adequately ballast the coupler and the resulting dye in the organic solvent in which the coupler is dispersed. The ballasting may be accomplished by providing hydrophobic substituent groups in one or more of the substituent groups. Generally a ballast group is an organic radical of such size and configuration as to confer on the coupler molecule sufficient bulk and aqueous insolubility as to render the coupler substantially nondiffusible from the layer in which it is coated in a photographic element. Thus the combination of substituent are suitably chosen to meet these criteria. To be effective, the ballast will usually contain at least 8 carbon atoms and typically contains 10 to 30 carbon atoms. Suitable

**29**

ballasting may also be accomplished by providing a plurality of groups which in combination meet these criteria. In the preferred embodiments of the invention  $R_1$  in formula (I) is a small alkyl group or hydrogen. Therefore, in these embodiments the ballast would be primarily located as part of the other groups. Furthermore, even if the coupling-off group  $Z$  contains a ballast it is often necessary to ballast the other substituents as well, since  $Z$  is eliminated from the molecule upon coupling; thus, the ballast is most advantageously provided as part of groups other than  $Z$ .  
<sup>5</sup>  
<sup>10</sup>

The following examples further illustrate preferred coupler of the invention. It is not to be construed that the present invention is limited to these examples.  
<sup>15</sup>



IC-1



IC-2



IC-3

**30**

-continued

IC-4



IC-5



IC-6



IC-7

**31**

-continued

**32**

-continued



**33**

-continued



IC-16

**34**

-continued



IC-20



IC-17



IC-21



IC-18



IC-22



IC-19



IC-23

**35**

-continued



IC-24

**36**

-continued

IC-27



IC-25 25



IC-28



IC-26 45



IC-29

60

65

**37**

-continued



IC-30

**38**

-continued



IC-33



IC-31



IC-34



IC-32



IC-35

**39**

-continued

**40**

Preferred couplers are IC-3, IC-7, IC-35, and IC-36 because of their suitably narrow left bandwidths.

Couplers that form magenta dyes upon reaction with oxidized color developing agent are described in such representative patents and publications as: U.S. Pat. Nos. 2,311,082, 2,343,703, 2,369,489, 2,600,788, 2,908,573, 3,062,653, 3,152,896, 3,519,429, 3,758,309, and "Farbkuppler-eine Literatur Ubersicht," published in Agfa Mitteilungen, Band III, pp. 126-156 (1961). Preferably such couplers are pyrazolones, pyrazolotriazoles, or pyrazolobenzimidazoles that form magenta dyes upon reaction with oxidized color developing agents. Especially preferred couplers are 1H-pyrazolo[5,1-c]-1,2,4-triazole and 1H-pyrazolo[1,5-b]-1,2,4-triazole. Examples of 1H-pyrazolo[5,1-c]-1,2,4-triazole couplers are described in U.K. Patent Nos. 1,247,493; 1,252,418; 1,398,979; U.S. Pat. Nos. 4,443,536; 4,514,490; 4,540,654; 4,590,153; 4,665,015; 4,822,730; 4,945,034; 5,017,465; and 5,023,170. Examples of 1H-pyrazolo[1,5-b]-1,2,4-triazoles can be found in European Patent applications 176,804; 177,765; U.S. Pat. Nos. 4,659,652; 5,066,575; and 5,250,400.

Typical pyrazolaoazole and pyrazolone couplers are represented by the following formulas:

MAGENTA-1



MAGENTA-2



wherein R<sub>a</sub> and R<sub>b</sub> independently represent H or a substituent; R<sub>c</sub> is a substituent (preferably an aryl group); R<sub>d</sub> is a substituent (preferably an anilino, carbonamido, ureido, carbamoyl, alkoxy, aryloxycarbonyl, alkoxy carbonyl, or N-heterocyclic group); X is hydrogen or a coupling-off group; and Z<sub>a</sub>, Z<sub>b</sub>, and Z<sub>c</sub> are independently a substituted methine group, =N=, =C=, or —NH—, provided that one of either the Z<sub>a</sub>—Z<sub>b</sub> bond or the Z<sub>b</sub>—Z<sub>c</sub> bond is a double bond and the other is a single bond, and when the Z<sub>b</sub>—Z<sub>c</sub> bond is a carbon-carbon double bond, it may form part of an aromatic ring, and at least one of Z<sub>a</sub>, Z<sub>b</sub>, and Z<sub>c</sub> represents a methine group connected to the group R<sub>b</sub>.

Specific examples of such couplers are:

M-1





Y-1



Y-2



Y-3



Y-4



Y-5



-continued



Unless otherwise specifically stated, substituent groups which may be substituted on molecules herein include any groups, whether substituted or unsubstituted, which do not destroy properties necessary for photographic utility. When the term "group" is applied to the identification of a substituent containing a substitutable hydrogen, it is intended to encompass not only the substituent's unsubstituted form, but also its form further substituted with any group or groups as herein mentioned. Suitably, the group may be halogen or may be bonded to the remainder of the molecule by an atom of carbon, silicon, oxygen, nitrogen, phosphorous, or sulfur. The substituent may be, for example, halogen, such as chlorine, bromine or fluorine; nitro; hydroxyl; cyano; carboxyl; or groups which may be further substituted, such as alkyl, including straight or branched chain alkyl, such as methyl, trifluoromethyl, ethyl, t-butyl, 3-(2,4-di-t-pentylphenoxy)propyl, and tetradecyl; alkenyl, such as ethylene, 2-butene; alkoxy, such as methoxy, ethoxy, propoxy, butoxy, 2-methoxyethoxy, sec-butoxy, hexyloxy, 2-ethylhexyloxy, tetradecyloxy, 2-(2,4-di-t-pentylphenoxy)ethoxy, and 2-dodecyloxyethoxy; aryl such as phenyl, 4-t-butylphenyl, 2,4,6-trimethylphenyl, naphthyl; aryloxy, such as phenoxy, 2-methylphenoxy, alpha- or beta-naphthoxy, and 4-tolyloxy; carbonamido, such as acetamido, benzamido, butyramido, tetradecanamido, alpha-(2,4-di-t-pentyl-phenoxy)acetamido, alpha-(2,4-di-t-pentylphenoxy)butyramido, alpha-(3-pentadecylphenoxy)-hexanamido, alpha-(4-hydroxy-3-t-butylphenoxy)-tetradecanamido, 2-oxo-pyrrolidin-1-yl, 2-oxo-5-tetradecylpyrrolin-1-yl, N-methyltetradecanamido, N-succinimido, N-phthalimido, 2,5-dioxo-1-oxazolidinyl, 3-dodecyl-2,5-dioxo-1-imidazolyl, and N-acetyl-N-dodecylamino, ethoxycarbonylamino, phenoxy carbonylamino, benzyloxy carbonylamino, hexadecyloxycarbonylamino, 2,4-di-t-butylphenoxy carbonylamino, phenyl carbonylamino, 2,5-(di-t-pentylphenyl) carbonylamino, p-dodecyl-phenyl carbonylamino, p-tolyl carbonylarnino, N-methylureido, N,N-dimethylureido, N-methyl-N-dodecylureido, N-hexadecylureido, N,N-dioctadecylureido, N,N-dioctyl-N'-ethylureido, N-phenylureido, N-phenylureido, N,N-diphenylureido, N-phenyl-N-p-tolylureido, N-(m-hexadecylphenyl)ureido, N,N-(2,5-di-t-pentylphenyl)-N'-ethylureido, and t-butyl carbonamido; sulfonamido, such as methylsulfonamido, benzenesulfonamido, p-tolylsulfonamido, p-dodecylbenzenesulfonamido, N-methyltetradecylsulfonamido, N,N-dipropylsulfamoylamino, and hexadecylsulfonamido; sulfamoyl, such as N-methylsulfamoyl, N-ethylsulfamoyl, N,N-

20 dipropylsulfamoyl, N-hexadecylsulfamoyl, N,N-dimethylsulfamoyl; N-[3-(dodecyloxy)propyl]sulfamoyl, N-[4-(2,4-di-t-pentylphenoxy)butyl]sulfamoyl, N-methyl-N-tetradecylsulfamoyl, and N-dodecylsulfamoyl; carbamoyl, such as N-methylcarbamoyl, N,N-dibutylcarbamoyl, N-octadecylcarbamoyl, N-[4-(2,4-di-t-pentylphenoxy)butyl]carbamoyl, N-methyl-N-tetradecylcarbamoyl, and N,N-diocetylcarbamoyl; acyl, such as acetyl, (2,4-di-t-amylphenoxy)acetyl, phenoxy carbonyl, p-dodecyloxyphenoxy carbonyl, methoxycarbonyl, butoxycarbonyl, tetradecyloxy carbonyl, ethoxycarbonyl, 30 benzoyloxy carbonyl, 3-pentadecyloxy carbonyl, and dodecylloxy carbonyl; sulfonyl, such as methoxysulfonyl, octyloxy sulfonfyl, tetradecyloxy sulfonfyl, 2-ethylhexyloxy sulfonfyl, phenoxy sulfonfyl, 2,4-di-t-pentylphenoxy sulfonfyl, methylsulfonyl, octylsulfonyl, 35 2-ethylhexylsulfonyl, dodecylsulfonyl, hexadecylsulfonyl, phenylsulfonyl, 4-nonylphenylsulfonyl, and p-tolylsulfonyl; sulfonyloxy, such as dodecylsulfonyloxy, and hexadecylsulfonyloxy; sulfinyl, such as methylsulfinyl, octylsulfinyl, 2-ethylhexylsulfinyl, dodecylsulfinyl, 40 hexadecylsulfinyl, phenylsulfinyl, 4-nonylphenylsulfinyl, and p-tolylsulfinyl; thio, such as ethylthio, octylthio, benzylthio, tetradecylthio, 2-(2,4-di-t-pentylphenoxy)ethylthio, phenylthio, 2-butoxy-5-t-octylphenylthio, and p-tolylthio; acyloxy, such as acyloxy, benzoyloxy, 45 octadecanoyloxy, p-dodecylamido benzoyloxy, N-phenylcarbamoyloxy, N-ethylcarbamoyloxy, and cyclohexylcarbonyloxy; amino, such as phenylanilino, 2-chloroanilino, diethylamino, dodecylamino; imino, such as 1 (N-phenylimido)ethyl, N-succinimido or 50 3-benzylhydantoinyl; phosphate, such as dimethylphosphate and ethylbutylphosphate; phosphite, such as diethyl and dihexylphosphite; a heterocyclic group, a heterocyclic oxy group or a heterocyclic thio group, each of which may be substituted and which contain a 3 to 7 membered heterocyclic ring composed of carbon atoms and at least one hetero atom selected from the group consisting of oxygen, nitrogen and sulfur, such as 2-furyl, 2-thienyl, 2-benzimidazolyl oxy or 2-benzothiazolyl; quaternary ammonium, such as triethylammonium; and silyloxy, such as trimethylsilyloxy.

60 If desired, the substituents may themselves be further substituted one or more times with the described substituent groups. The particular substituents used may be selected by those skilled in the art to attain the desired photographic properties for a specific application and can include, for 65 example, hydrophobic groups, solubilizing groups, blocking groups, releasing or releasable groups, etc. Generally, the above groups and substituents thereof may include those

**47**

having up to 48 carbon atoms, typically 1 to 36 carbon atoms and usually less than 24 carbon atoms, but greater numbers are possible depending on the particular substituents selected.

Representative substituents on ballast groups include alkyl, aryl, alkoxy, aryloxy, alkylthio, hydroxy, halogen, alkoxycarbonyl, arylox carbonyl, carboxy, acyl, acyloxy,

**48**

amino, anilino, carbonamido, carbamoyl, alkylsulfonyl, arylsulfonyl, sulfonamido, and sulfamoyl groups wherein the substituents typically contain 1 to 42 carbon atoms. Such substituents can also be further substituted.

Stabilizers and scavengers that can be used in these photographic elements, but are not limited to, the following.

ST-1



ST-2



ST-3



ST-4



ST-5



ST-6



ST-7



ST-8



ST-9





-continued

ST-10



ST-11



ST-12



ST-13

ST-14



ST-15



ST-16



ST-17



ST-18

51



-continued

ST-19



ST-20



ST-21



ST-22



ST-23



ST-24

Examples of solvents which may be used in the invention include the following:

35

-continued

|                                   |     |
|-----------------------------------|-----|
| Tritolyl phosphate                | S-1 |
| Dibutyl phthalate                 | S-2 |
| Diundecyl phthalate               | S-3 |
| N,N-Diethyldodecanamide           | S-4 |
| N,N-Dibutyldodecanamide           | S-5 |
| Tris(2-ethylhexyl)phosphate       | S-6 |
| Acetyl tributyl citrate           | S-7 |
| 2,4-Di- <i>tert</i> -pentylphenol | S-8 |

2-(2-Butoxyethoxy)ethyl acetate  
1,4-Cyclohexyldimethylene bis(2-ethylhexanoate)

S-9

S-10

40

The dispersions used in photographic elements may also include ultraviolet (UV) stabilizers and so called liquid UV stabilizers such as described in U.S. Pat. Nos. 4,992,358; 4,975,360; and 4,587,346. Examples of UV stabilizers are shown below.

UV-1



-1

UV-2



53

54

-continued

UV-3



UV-5



UV 3



The aqueous phase may include surfactants. Surfactants may be cationic, anionic, zwitterionic or non-ionic. Useful surfactants include, but are not limited to, the following:

30



$\text{CH}_2\text{-}(\text{CH}_2)_n\text{-SO}_3\text{Na}$ ,  $n = 12-14$



SE-2



SE-5

SE-6



n = ca. 10



$\eta \approx \text{ca. } 40$



n = ca. 6, m = ca. 2



Further, it is contemplated to stabilize photographic dispersions prone to particle growth through the use of hydrophobic, photographically inert compounds such as disclosed by Zengerle et al in U.S. Pat. No. 5,468,604.

The photographic elements may also contain filter dye layers comprising colloidal silver sol or yellow, cyan, and/or magenta filter dyes, either as oil-in-water dispersions, latex dispersions or as solid particle dispersions. Useful examples of absorbing materials are discussed in *Research Disclosure*, September 1996, Item 38957, Section VIII.

-continued

SF-9



SF-11



The photographic elements may also contain light absorbing materials that can increase sharpness and be used to control speed and minimum density. Examples of useful absorber dyes are described in U.S. Pat. Nos. 4,877,721; 5,001,043; 5,153,108; and 5,035,985. Solid particle dispersion dyes are described in U.S. Pat. Nos. 4,803,150; 4,855,221; 4,857,446; 4,900,652; 4,900,653; 4,940,654; 4,948,717; 4,948,718; 4,950,586; 4,988,611; 4,994,356; 5,098,820; 5,213,956; 5,260,179; and 5,266,454. Useful dyes include, but are not limited to, the following.

DYE-1



DYE-2



DYE-3



DYE-4





-continued

DYE-8



DYE-9



30

In a preferred embodiment the invention employs recording elements which are constructed to contain at least three silver halide emulsion layer units. A suitable full color, multilayer format for a recording element used in the invention is represented by Structure I.

| STRUCTURE I       |                                                       |
|-------------------|-------------------------------------------------------|
| Red-sensitized    | cyan dye image-forming silver halide emulsion unit    |
| Interlayer        |                                                       |
| Green-sensitized  | magenta dye image-forming silver halide emulsion unit |
| Interlayer        |                                                       |
| Blue-sensitized   | yellow dye image-forming silver halide emulsion unit  |
| //// Support //// |                                                       |

wherein the red-sensitized, cyan dye image-forming silver halide emulsion unit is situated nearest the support; next in order is the green-sensitized, magenta dye image-forming unit, followed by the uppermost blue-sensitized, yellow dye image-forming unit. The image-forming units are separated from each other by hydrophilic colloid interlayers containing an oxidized developing agent scavenger to prevent color contamination. Silver halide emulsions satisfying the grain and gelatino-peptizer requirements described above can be present in any one or combination of the emulsion layer units. Additional useful multicolor, multilayer formats for an element of the invention include structures as described in U.S. Pat. No. 5,783,373. Each of such structures in accordance with the invention preferably would contain at least three silver halide emulsions comprised of high chloride

grains having at least 50 percent of their surface area bounded by {100} crystal faces and containing dopants from classes (i) and (ii), as described above. Preferably each of the emulsion layer units contains emulsion satisfying these criteria.

In a more preferred embodiment, the invention employs recording elements which are constructed as described in U.S. Pat. No. 5,948,601 of Rieger. In this embodiment, the invention employs recording elements which are constructed to contain at least three silver halide emulsion layer units and an interlayer adjacent to the blue sensitive emulsion layer

Conventional features that can be incorporated into multilayer (and particularly multicolor) recording elements contemplated for use in the method of the invention are illustrated by *Research Disclosure*, Item 38957, cited above:

## XI. Layers and layer arrangements

## XII. Features applicable only to color negative

## XIII. Features applicable only to color positive

## B. Color reversal

## C. Color positives derived from color negatives

## XIV. Scan facilitating features.

The recording elements comprising the radiation sensitive high chloride emulsion layers according to this invention can be conventionally optically printed, or in accordance with a particular embodiment of the invention can be image-wise exposed in a pixel-by-pixel mode using suitable high energy radiation sources typically employed in electronic printing methods. Suitable actinic forms of energy encompass the ultraviolet, visible and infrared regions of the electromagnetic spectrum as well as electron-beam radiation and is conveniently supplied by beams from one or more light emitting diodes or lasers, including gaseous or solid state lasers. Exposures can be monochromatic, orthochromatic or panchromatic. For example, when the recording element is a multilayer multicolor element, exposure can be provided by laser or light emitting diode beams of appro-

priate spectral radiation, for example, infrared, red, green or blue wavelengths, to which such element is sensitive. Multicolor elements can be employed which produce cyan, magenta, and yellow dyes as a function of exposure in separate portions of the electromagnetic spectrum, including at least two portions of the infrared region, as disclosed in the previously mentioned U.S. Pat. No. 4,619,892. Suitable exposures include those up to 2000 nm, preferably up to 1500 nm. Suitable light emitting diodes and commercially available laser sources are known and commercially available. Imagewise exposures at ambient, elevated or reduced temperatures and/or pressures can be employed within the useful response range of the recording element determined by conventional sensitometric techniques, as illustrated by T. H. James, *The Theory of the Photographic Process*, 4th Ed., Macmillan, 1977, Chapters 4, 6, 17, 18 and 23.

It has been observed that anionic  $[MX_xY_yL_z]$  hexacoordination complexes, where M is a group 8 or 9 metal (preferably iron, ruthenium or iridium), X is halide or pseudohalide (preferably Cl, Br or CN) x is 3 to 5, Y is  $H_2O$ , y is 0 or 1, L is a C—C, H—C or C—N—H organic ligand, and Z is 1 or 2, are surprisingly effective in reducing high intensity reciprocity failure (HIRF), low intensity reciprocity failure (LIRF) and thermal sensitivity variance and in improving latent image keeping (LIK). As herein employed HIRF is a measure of the variance of photographic properties for equal exposures, but with exposure times ranging from  $10^{-1}$  to  $10^{-6}$  second. LIRF is a measure of the variance of photographic properties for equal exposures, but with exposure times ranging from  $10^{-1}$  to 100 seconds. Although these advantages can be generally compatible with face centered cubic lattice grain structures, the most striking improvements have been observed in high (>50 mole %, preferably  $\geq 90$  mole %) chloride emulsions. Preferred C—C, H—C or C—N—H organic ligands are aromatic heterocycles of the type described in U.S. Pat. No. 5,462,849. The most effective C—C, H—C or C—N—H organic ligands are azoles and azines, either unsubstituted or containing alkyl, alkoxy or halide substituents, where the alkyl moieties contain from 1 to 8 carbon atoms. Particularly preferred azoles and azines include thiazoles, thiazolines, and pyrazines.

The quantity or level of high energy actinic radiation provided to the recording medium by the exposure source is generally at least  $10^{-4}$  ergs/cm<sup>2</sup>, typically in the range of about  $10^{-4}$  ergs/cm<sup>2</sup> to  $10^{-3}$  ergs/cm<sup>2</sup> and often from  $10^{-3}$  ergs/cm<sup>2</sup> to  $10^2$  ergs/cm<sup>2</sup>. Exposure of the recording element in a pixel-by-pixel mode as known in the prior art persists for only a very short duration or time. Typical maximum exposure times are up to  $100\mu$  seconds, often up to  $10\mu$  seconds, and frequently up to only  $0.5\mu$  seconds. Single or multiple exposures of each pixel are contemplated. The pixel density is subject to wide variation, as is obvious to those skilled in the art. The higher the pixel density, the sharper the images can be, but at the expense of equipment complexity. In general, pixel densities used in conventional electronic printing methods of the type described herein do not exceed  $10^7$  pixels/cm<sup>2</sup> and are typically in the range of about  $10^4$  to  $10^6$  pixels/cm<sup>2</sup>. An assessment of the technology of high-quality, continuous-tone, color electronic printing using silver halide photographic paper which discusses various features and components of the system, including exposure source, exposure time, exposure level and pixel density and other recording element characteristics is provided in Firth et al., *A Continuous-Tone Laser Color Printer*, Journal of Imaging Technology, Vol. 14, No. 3, June 1988. As previously indicated herein, a description of some of the details

of conventional electronic printing methods comprising scanning a recording element with high energy beams such as light emitting diodes or laser beams, are set forth in Hioki U.S. Pat. No. 5,126,235, European Patent Applications 479 167 A1 and 502 508 A1.

Once imagewise exposed, the recording elements can be processed in any convenient conventional manner to obtain a viewable image. Such processing is illustrated by *Research Disclosure*, Item 38957, cited above:

XVIII. Chemical development systems

XIX. Development

XX. Desilvering, washing, rinsing and stabilizing.

In addition, a useful developer for the inventive material is a homogeneous, single part developing agent. The homogeneous, single-part color developing concentrate is prepared using a critical sequence of steps:

In the first step, an aqueous solution of a suitable color developing agent is prepared. This color developing agent is generally in the form of a sulfate salt. Other components of the solution can include an antioxidant for the color developing agent, a suitable number of alkali metal ions (in an at least stoichiometric proportion to the sulfate ions) provided by an alkali metal base, and a photographically inactive water-miscible or water-soluble hydroxy-containing organic solvent. This solvent is present in the final concentrate at a concentration such that the weight ratio of water to the organic solvent is from about 15:85 to about 50:50.

In this environment, especially at high alkalinity, alkali metal ions and sulfate ions form a sulfate salt that is precipitated in the presence of the hydroxy-containing organic solvent. The precipitated sulfate salt can then be readily removed using any suitable liquid/solid phase separation technique (including filtration, centrifugation or decantation). If the antioxidant is a liquid organic compound, two phases may be formed and the precipitate may be removed by discarding the aqueous phase.

The color developing concentrates of this invention include one or more color developing agents that are well known in the art that, in oxidized form, will react with dye forming color couplers in the processed materials. Such color developing agents include, but are not limited to, aminophenols, p-phenylenediamines (especially N,N-dialkyl-p-phenylenediamines) and others which are well known in the art, such as EP 0 434 097 A1 (published Jun. 26, 1991) and EP 0 530 921 A1 (published Mar. 10, 1993). It may be useful for the color developing agents to have one or more water-solubilizing groups as are known in the art. Further details of such materials are provided in *Research Disclosure*, publication 38957, pages 592-639 (September 1996). *Research Disclosure* is a publication of Kenneth Mason Publications Ltd., Dudley House, 12 North Street, Emsworth, Hampshire PO10 7DQ England (also available from Emsworth Design Inc., 121 West 19th Street, New York, N.Y. 10011).

Preferred color developing agents include, but are not limited to, N,N-diethyl p-phenylenediamine sulfate (KODAK Color Developing Agent CD-2), 4-amino-3-methyl-N-(2-methane sulfonamidoethyl)aniline-sulfate, 4-(N-ethyl-N-β-hydroxyethylamino)-2-methylaniline sulfate (KODAK Color Developing Agent CD-4), p-hydroxyethylaminoaniline sulfate, 4-(N-ethyl-N-2-methanesulfonylaminooethyl)-2-methylphenylenediamine sesquisulfate (KODAK Color Developing Agent CD-3), 4-(N-ethyl-N-2-methanesulfonylaminooethyl)-2-methylphenylenediamine sesquisulfate, and others readily apparent to one skilled in the art.

In order to protect the color developing agents from oxidation, one or more antioxidants are generally included

in the color developing compositions. Either inorganic or organic antioxidants can be used. Many classes of useful antioxidants are known, including but not limited to, sulfites (such as sodium sulfite, potassium sulfite, sodium bisulfite and potassium metabisulfite), hydroxylamine (and derivatives thereof), hydrazines, hydrazides, amino acids, ascorbic acid (and derivatives thereof), hydroxamic acids, aminoketones, mono- and polysaccharides, mono- and polyamines, quaternary ammonium salts, nitroxy radicals, alcohols, and oximes. Also useful as antioxidants are 1,4-cyclohexadienes. Mixtures of compounds from the same or different classes of antioxidants can also be used if desired.

Especially useful antioxidants are hydroxylamine derivatives as described, for example, in U.S. Pat. Nos. 4,892,804; 4,876,174; 5,354,646; and 5,660,974, all noted above, and U.S. Pat. No. 5,646,327 (Bums et al). Many of these antioxidants are mono- and dialkylhydroxylamines having one or more substituents on one or both alkyl groups. Particularly useful alkyl substituents include sulfo, carboxy, amino, sulfonamido, carbonamido, hydroxy and other solubilizing substituents.

More preferably, the noted hydroxylamine derivatives can be mono- or dialkylhydroxylamines having one or more hydroxy substituents on the one or more alkyl groups. Representative compounds of this type are described for example in U.S. Pat. No. 5,709,982 (Marrese et al) as having the structure I:



wherein R is hydrogen, a substituted or unsubstituted alkyl group of 1 to 10 carbon atoms, a substituted or unsubstituted hydroxyalkyl group of 1 to 10 carbon atoms, a substituted or unsubstituted cycloalkyl group of 5 to 10 carbon atoms, or a substituted or unsubstituted aryl group having 6 to 10 carbon atoms in the aromatic nucleus.

$\text{X}_1$  is  $-\text{CR}_2(\text{OH})\text{CHR}_1-$  and  $\text{X}_2$  is  $-\text{CHR}_1\text{CR}_2(\text{OH})-$  wherein  $\text{R}_1$  and  $\text{R}_2$  are independently hydrogen, hydroxy, a substituted or unsubstituted alkyl group of 1 or 2 carbon atoms, a substituted or unsubstituted hydroxyalkyl group of 1 or 2 carbon atoms, or  $\text{R}_1$  and  $\text{R}_2$  together represent the carbon atoms necessary to complete a substituted or unsubstituted 5- to 8-membered saturated or unsaturated carbocyclic ring structure.

$\text{Y}$  is a substituted or unsubstituted alkylene group having at least 4 carbon atoms, and has an even number of carbon atoms, or  $\text{Y}$  is a substituted or unsubstituted divalent aliphatic group having an even total number of carbon and oxygen atoms in the chain, provided that the aliphatic group has a least 4 atoms in the chain.

Also in Structure I, m, n and p are independently 0 or 1. Preferably, each of m and n is 1, and p is 0.

Specific di-substituted hydroxylamine antioxidants include, but are not limited to: N,N-bis(2,3-dihydroxypropyl)hydroxylamine, N,N-bis(2-methyl-2,3-dihydroxypropyl)hydroxylamine and N,N-bis(1-hydroxymethyl-2-hydroxy-3-phenylpropyl)hydroxylamine. The first compound is preferred.

The following examples illustrate the practice of this invention. They are not intended to be exhaustive of all possible variations of the invention. Parts and percentages are by weight unless otherwise indicated.

## EXAMPLES

### Example 1

In this example the color silver halide emulsion of the invention was coated on two imaging support materials. The

first support material of the invention was constructed by laminating biaxially oriented sheets to cellulose photographic grade paper. The second support material, which is the control material, was constructed by melt extrusion coating with low density polyethylene cellulose photographic grade paper. The control material is typical of prior art photographic support materials. This example will show the improvement the invention has made compared to the control in digital printing. Further, this example will also demonstrate the image sharpness, whiteness, and durability improvement over prior art photographic base materials.

The support material utilized in the control consisted of melt extruded low density polyethylene applied to a photographic grade cellulose paper base. The low density polyethylene on the topside of the control support contains blue tint, anatase  $\text{TiO}_2$  and optical brightener. The control support structure is typical of prior art color photographic base materials.

The following is a description of the invention and was prepared by extrusion laminating the following top and bottom biaxially oriented sheets to the photographic grade cellulose paper described below:

#### Top Sheet (Emulsion Side)

A composite sheet consisting of 5 layers identified as L1, L2, L3, L4, and L5. L1 is the thin colored layer on the outside of the package to which the photosensitive silver halide layer was attached. L2 is the layer to which optical brightener and  $\text{TiO}_2$  was added. The optical brightener used was Hostalux KS manufactured by Ciba-Geigy. A coated extrusion grade anatase  $\text{TiO}_2$  was added to both L2 and L4. Table 1 below lists the characteristics of the layers of the top biaxially oriented sheet used in this example.

TABLE 1

| Layer | Material                                | Thickness, $\mu\text{m}$ |
|-------|-----------------------------------------|--------------------------|
| L1    | LD Polyethylene + color concentrate     | 0.65                     |
| L2    | Polypropylene + 24% $\text{TiO}_2$ + OB | 6.75                     |
| L3    | Voided Polypropylene                    | 30                       |
| L4    | Polypropylene + 18% $\text{TiO}_2$      | 6.90                     |
| L5    | Polypropylene                           | 0.66                     |

#### Photographic Grade Cellulose Paper Base Used in the Invention

Paper base was produced for the invention using a standard fourdrinier paper machine and a blend of mostly bleached hardwood Kraft fibers. The fiber ratio consisted primarily of bleached poplar (38%) and maple/beech (37%) with lesser amounts of birch (18%) and softwood (7%). Fiber length was reduced from 0.73 mm length weighted average as measured by a Kajaani FS-200 to 0.55 mm length using high levels of conical refining and low levels of disc refining. Fiber lengths from the slurry were measured using an FS-200 Fiber Length Analyzer (Kajaani Automation Inc.). Energy applied to the fibers is indicated by the total Specific Net Refining Power (SNRP) was 127 KW hr/metric ton. Two conical refiners were used in series to provide the total conical refiners SNRP value. This value was obtained by adding the SNRPs of each conical refiner. Two disc refiners were similarly used in series to provide a total Disk SNRP. Neutral sizing chemical addenda, utilized on a dry weight basis, included alkyl ketene dimer at 0.20% addition, cationic starch (1.0%), polyaminoamide epichlorhydrin (0.50%), polyacrylamide resin (0.18%), diaminostilbene optical brightener (0.20%), and sodium bicarbonate. Surface sizing using hydroxyethylated starch and sodium chloride was also employed but is not critical to the invention. In the

3<sup>rd</sup> Dryer section, ratio drying was utilized to provide a moisture bias from the face side to the wire side of the sheet. The face side (emulsion side) of the sheet was then remoisturized with conditioned steam immediately prior calendering. Sheet temperatures were raised to between 76° C. and 93° C. just prior to and during calendering. The paper was then calendered to an apparent density of 1.17. Moisture levels after the calender were 7.0% to 9.0% by weight. Paper base B was produced at a thickness of 254 micrometers.

Bottom Sheet (Backside)

The bottom biaxially oriented sheet laminated to the backside of invention base was a one-side matte finish, biaxially oriented polypropylene sheet (25.6  $\mu\text{m}$  thick) ( $d=0.90 \text{ g/cc}$ ) consisting of a solid oriented polypropylene layer and a skin layer of a mixture of polyethylenes and a terpolymer comprising ethylene, propylene, and butylene. The skin layer was on the bottom, and the polypropylene layer was laminated to the paper.

The top sheet used in this example was coextruded and biaxially oriented. The top sheet was melt extrusion laminated to the above cellulose paper base using a metallocene catalyzed ethylene plastomer (SLP 9088) manufactured by Exxon Chemical Corp. The metallocene catalyzed ethylene plastomer had a density of 0.900  $\text{g/cc}$  and a melt index of 14.0.

A coating was then applied to the laminated bottom biaxially oriented sheet on invention using a gravure coater to add the high frequency roughness to the backside. The coating consisted of an aqueous solution containing a sodium salt of styrene sulfonic acid dispersed in an acrylate latex. The coverage used was 25 mg per square meter and then dried to achieve a final web temperature between 55° C., the resultant coalesced latex material produced the desired high frequency roughness pattern. In addition to the sodium salt of styrene sulfonic acid, aluminum modified colloidal silicon dioxide particles were added to the aqueous latex material at a concentration of 50 milligrams per square meter. This further enhanced the high frequency roughness.

The L3 layer for the biaxially oriented sheet is microvoided and further described in Table 2 where the refractive index and geometrical thickness is shown for measurements made along a single slice through the L3 layer; they do not imply continuous layers, a slice along another location would yield different but approximately the same thickness. The areas with a refractive index of 1.0 are voids that are filled with air and the remaining layers are polypropylene.

TABLE 2

| Sublayer of L3 | Refractive Index | Thickness, $\mu\text{m}$ |
|----------------|------------------|--------------------------|
| 1              | 1.49             | 2.54                     |
| 2              | 1                | 2.027                    |
| 3              | 1.49             | 2.79                     |
| 4              | 1                | 2.016                    |
| 5              | 1.49             | 1.778                    |
| 6              | 1                | 2.016                    |
| 7              | 1.49             | 2.286                    |
| 8              | 1                | 2.016                    |
| 9              | 1.49             | 2.032                    |
| 10             | 1                | 0.762                    |
| 11             | 1.49             | 2.032                    |
| 12             | 1                | 2.016                    |
| 13             | 1.49             | 2.278                    |
| 14             | 1                | 2.016                    |
| 15             | 1.49             | 2.286                    |

Silver chloride emulsions were chemically and spectrally sensitized as described below. A biocide comprising a mixture of N-methyl-isothiazolone and N-methyl-5-chloro-isothiazolone was added after sensitization.

Blue Sensitive Emulsion (Blue EM-1). A high chloride silver halide emulsion is precipitated by adding approximately equimolar silver nitrate and sodium chloride solutions into a well-stirred reactor containing p-glutarylaminophenylsulfide, gelatin peptizer, and thioether ripener. Cesium pentachloronitrosylsulfate(II) dopant is added during the silver halide grain formation from 3.9% to 70% of the making process, followed by the addition of potassium hexacyanoruthenate(II) at 75–80% of the make and potassium (5-methylthiazole)-pentachloroiodate from 92–95% of the make. In addition, potassium iodide was added at 90%+/-3% of the making process to form a band of silver iodide at 0.2%+/-0.1% of the silver in the grain. The resultant emulsion contains cubic shaped grains having edge length of 0.64  $\mu\text{m}$ . The emulsion is optimally sensitized by the addition of p-glutarylaminophenylsulfide followed by a colloidal suspension of aurous sulfide and heat ramped to 60° C. After the temperature reached 60° C., blue sensitizing dye BSD-4, potassium hexachloroiodate, Lippmann bromide, and 1-(3-acetamidophenyl)-5-mercaptotetrazole were added.

Green Sensitive Emulsion (Green EM-1): A high chloride silver halide emulsion is precipitated by adding approximately equimolar silver nitrate and sodium chloride solutions, the silver nitrate solution containing p-glutarylaminophenylsulfide, into a well-stirred reactor containing gelatin peptizer and thioether ripener. Cesium pentachloronitrosylsulfate(II) dopant is added from 1.5% to 75% of the silver halide grain formation, followed by the addition of potassium (5-methylthiazole)-pentachloroiodate from 90–95% of the precipitation. The resultant emulsion contains cubic shaped grains of 0.34  $\mu\text{m}$  in edgelength size. The emulsion is optimally sensitized by the addition of a liquid crystalline suspension of green sensitizing dye GSD-1 and a colloidal suspension of aurous sulfide followed by heating to 60° C. for 35 minutes. After cooling to 40° C., an antifoggant 1-(3-acetamidophenyl)-5-mercaptotetrazole, potassium bromide, and potassium chloride were added.

Red Sensitive Emulsion (Red EM-1): A high chloride silver halide emulsion is precipitated by adding approximately equimolar silver nitrate and sodium chloride solutions into a well-stirred reactor containing gelatin peptizer and thioether ripener. During the silver halide grain formation, cesium pentachloronitrosylsulfate, potassium hexacyanoruthenate(II) and potassium (5-methylthiazole)-pentachloroiodate are added from 3–75%, 80–85% and 90–95% of the precipitation, respectively. The resultant emulsion contains cubic shaped grains of 0.38  $\mu\text{m}$  in edgelength size. The emulsion is optimally sensitized by the addition of glutarylaminophenylsulfide, sodium thiosulfate and Bis (1,4,5-trimethyl-1,2,4-triazolium-3-thiolate)gold(I) fluoroborate. After heating to 65° C. this emulsion was held for 28 minutes, and then the following were added: 1-(3-acetamidophenyl)-5-mercaptotetrazole, potassium hexachloroiodate, and potassium bromide. The emulsion is then cooled to 40° C. and red sensitizing dye RSD-1 is added.

Coupler dispersions were emulsified by methods well known to the art, and the following layers were coated on the following support:

The following light sensitive silver halide imaging layers were utilized to prepare photographic print materials for the invention. The following imaging layers were coated utilizing curtain coating.

-continued

| Item                                             | Laydown g/m <sup>2</sup> | Item                                                                         | Laydown g/m <sup>2</sup> |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
|--------------------------------------------------|--------------------------|------------------------------------------------------------------------------|--------------------------|--------------------------------|--------|---------------------------------|--------|-------------------------|--------|-------------------------------|--------|-------------|--------|------|--------|----------------------|--------|------|--------|---------------------------------------------------------------------------|--------|-----|--------|---------------------------------------------------------------------------|--------|-------------|--------|---------|--------|--------------------------------|--------|---------------------------------|--------|------------------------------|--------|-------------------------------|--------|--------------------------|--------|-------|--------|---------------------|--|---------|--------|------|--------|------|--------|------------------|--------|------|--------|-----|--------|------|--------|-------|--------|------|--------|----------------------------------|--------|-----|--------|---------------------------------------------------------------------------|--------|-------------|--|---------|--------|--------------------------------|--------|------------------------------|--------|------|--------|-------------------------------|--------|--|--|
| Layer 1 Blue Sensitive Layer                     |                          | 5 Layer 1 Blue Sensitive Layer                                               |                          |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Gelatin                                          | 1.3885                   | Gelatin                                                                      | 1.3127                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Blue Sensitive silver (Blue EM-1)                | 0.2799                   | Blue sensitive silver (Blue EM-1)                                            | 0.2399                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Y-5                                              | 0.4521                   | Y-4                                                                          | 0.4143                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| ST-6                                             | 0.0775                   | ST-23                                                                        | 0.4842                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| ST-7                                             | 0.0258                   | Tributyl Citrate                                                             | 0.2179                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| S-3                                              | 0.1981                   | ST-24                                                                        | 0.1211                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Piperidino hexose reductone                      | 0.0023                   | ST-16                                                                        | 0.0095                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Sodium phenylmercaptotetrazole                   | 0.0001                   | Sodium Phenylmercaptotetrazole                                               | 0.0001                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| DYE-1                                            | 0.0323                   | Piperidino hexose reductone                                                  | 0.0024                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Layer 2 Split Yellow Interlayer                  |                          | 15 5-chloro-2-methyl-4-isothiazolin-3-one/2-methyl-4-isothiazolin-3-one(3/1) | 0.0002                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Gelatin                                          | 0.3229                   | SF-1                                                                         | 0.0366                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Y-5                                              | 0.1938                   | Potassium chloride                                                           | 0.0204                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| ST-6                                             | 0.0332                   | Dye-1                                                                        | 0.0148                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| ST-7                                             | 0.0111                   | Layer 2 Interlayer                                                           |                          |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| S-3                                              | 0.0849                   | Gelatin                                                                      | 0.7532                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Layer 3 Interlayer                               |                          | ST-4                                                                         | 0.1076                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Gelatin                                          | 0.7535                   | S-3                                                                          | 0.1969                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| ST-4                                             | 0.0660                   | 5-chloro-2-methyl-4-isothiazolin-3-one/2-methyl-4-isothiazolin-3-one(3/1)    | 0.0001                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| S-2                                              | 0.1884                   | Catechol disulfonate                                                         | 0.0323                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Acrylamide/t-Butylacrylamide sulfonate copolymer | 0.1281                   | SF-1                                                                         | 0.0081                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Bis-vinylsulfonylmethane                         | 0.0151                   | Layer 3 Green Sensitive Layer                                                |                          |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Layer 4 Green Sensitive Layer                    |                          | Gelatin                                                                      | 1.1944                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Gelatin                                          | 1.3498                   | 1)                                                                           | 0.1011                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Green Sensitive silver (Green EM-1)              | 0.1076                   | M-4                                                                          | 0.2077                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| M-2                                              | 0.2142                   | Oleyl Alcohol                                                                | 0.2174                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| S-2                                              | 0.0761                   | S-3                                                                          | 0.1119                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| S-3                                              | 0.0326                   | ST-21                                                                        | 0.0398                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| ST-8                                             | 0.0560                   | ST-22                                                                        | 0.2841                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| ST-21                                            | 0.1636                   | Dye-2                                                                        | 0.0073                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| DYE-2                                            | 0.0075                   | 5-chloro-2-methyl-4-isothiazolin-3-one/2-methyl-4-isothiazolin-3-one(3/1)    | 0.0001                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Sodium phenylmercaptotetrazole                   | 0.0003                   | SF-1                                                                         | 0.0236                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Layer 5 UV Interlayer                            |                          | Potassium chloride                                                           | 0.0204                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Gelatin                                          | 0.7136                   | Sodium Phenylmercaptotetrazole                                               | 0.0007                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| UV-1                                             | 0.0312                   | Layer 4 M/C Interlayer                                                       |                          |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| UV-2                                             | 0.1722                   | Gelatin                                                                      | 0.7532                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| ST-4                                             | 0.0527                   | ST-4                                                                         | 0.1076                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| S-10                                             | 0.0344                   | S-3                                                                          | 0.1969                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| S-2                                              | 0.0344                   | Acrylamide/t-Butylacrylamide sulfonate copolymer                             | 0.0541                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Layer 6 Red Sensitive Layer                      |                          | Gelatin                                                                      | 1.3563                   | Bis-vinylsulfonylmethane       | 0.1390 | Red sensitive silver (Red EM-1) | 0.1938 | 3,5-Dinitrobenzoic acid | 0.0001 | C-1                           | 0.4004 | Citric acid | 0.0007 | S-2  | 0.3918 | Catechol disulfonate | 0.0323 | UV-2 | 0.2573 | 5-chloro-2-methyl-4-isothiazolin-3-one/2-methyl-4-isothiazolin-3-one(3/1) | 0.0001 | S-9 | 0.0328 | Layer 5 Red Sensitive Layer                                               |        | ST-4        | 0.0033 | Gelatin | 1.3558 | DYE-3                          | 0.0151 | Red Sensitive silver (Red EM-1) | 0.1883 | Potassium tolylthiosulfonate | 0.0027 | IC-35                         | 0.2324 | Potassium tolylsulfonate | 0.0003 | IC-36 | 0.0258 | Layer 7 UV Overcoat |  | Gelatin | 0.5350 | UV-2 | 0.3551 | UV-1 | 0.0229 | Dibutyl sebacate | 0.4358 | UV-2 | 0.1301 | S-6 | 0.1453 | ST-4 | 0.0384 | Dye-3 | 0.0229 | S-10 | 0.0255 | Potassium p-toluenethiosulfonate | 0.0026 | S-2 | 0.0255 | 5-chloro-2-methyl-4-isothiazolin-3-one/2-methyl-4-isothiazolin-3-one(3/1) | 0.0001 | Layer 8 SOC |  | Gelatin | 0.6458 | Sodium Phenylmercaptotetrazole | 0.0005 | Ludox AM™ (colloidal silica) | 0.1615 | SF-1 | 0.0524 | Polydimethylsiloxane (DC200™) | 0.0202 |  |  |
| Gelatin                                          | 1.3563                   | Bis-vinylsulfonylmethane                                                     | 0.1390                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Red sensitive silver (Red EM-1)                  | 0.1938                   | 3,5-Dinitrobenzoic acid                                                      | 0.0001                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| C-1                                              | 0.4004                   | Citric acid                                                                  | 0.0007                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| S-2                                              | 0.3918                   | Catechol disulfonate                                                         | 0.0323                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| UV-2                                             | 0.2573                   | 5-chloro-2-methyl-4-isothiazolin-3-one/2-methyl-4-isothiazolin-3-one(3/1)    | 0.0001                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| S-9                                              | 0.0328                   | Layer 5 Red Sensitive Layer                                                  |                          |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| ST-4                                             | 0.0033                   | Gelatin                                                                      | 1.3558                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| DYE-3                                            | 0.0151                   | Red Sensitive silver (Red EM-1)                                              | 0.1883                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Potassium tolylthiosulfonate                     | 0.0027                   | IC-35                                                                        | 0.2324                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Potassium tolylsulfonate                         | 0.0003                   | IC-36                                                                        | 0.0258                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Layer 7 UV Overcoat                              |                          | Gelatin                                                                      | 0.5350                   | UV-2                           | 0.3551 | UV-1                            | 0.0229 | Dibutyl sebacate        | 0.4358 | UV-2                          | 0.1301 | S-6         | 0.1453 | ST-4 | 0.0384 | Dye-3                | 0.0229 | S-10 | 0.0255 | Potassium p-toluenethiosulfonate                                          | 0.0026 | S-2 | 0.0255 | 5-chloro-2-methyl-4-isothiazolin-3-one/2-methyl-4-isothiazolin-3-one(3/1) | 0.0001 | Layer 8 SOC |        | Gelatin | 0.6458 | Sodium Phenylmercaptotetrazole | 0.0005 | Ludox AM™ (colloidal silica)    | 0.1615 | SF-1                         | 0.0524 | Polydimethylsiloxane (DC200™) | 0.0202 |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Gelatin                                          | 0.5350                   | UV-2                                                                         | 0.3551                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| UV-1                                             | 0.0229                   | Dibutyl sebacate                                                             | 0.4358                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| UV-2                                             | 0.1301                   | S-6                                                                          | 0.1453                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| ST-4                                             | 0.0384                   | Dye-3                                                                        | 0.0229                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| S-10                                             | 0.0255                   | Potassium p-toluenethiosulfonate                                             | 0.0026                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| S-2                                              | 0.0255                   | 5-chloro-2-methyl-4-isothiazolin-3-one/2-methyl-4-isothiazolin-3-one(3/1)    | 0.0001                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Layer 8 SOC                                      |                          | Gelatin                                                                      | 0.6458                   | Sodium Phenylmercaptotetrazole | 0.0005 | Ludox AM™ (colloidal silica)    | 0.1615 | SF-1                    | 0.0524 | Polydimethylsiloxane (DC200™) | 0.0202 |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Gelatin                                          | 0.6458                   | Sodium Phenylmercaptotetrazole                                               | 0.0005                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Ludox AM™ (colloidal silica)                     | 0.1615                   | SF-1                                                                         | 0.0524                   |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |
| Polydimethylsiloxane (DC200™)                    | 0.0202                   |                                                                              |                          |                                |        |                                 |        |                         |        |                               |        |             |        |      |        |                      |        |      |        |                                                                           |        |     |        |                                                                           |        |             |        |         |        |                                |        |                                 |        |                              |        |                               |        |                          |        |       |        |                     |  |         |        |      |        |      |        |                  |        |      |        |     |        |      |        |       |        |      |        |                                  |        |     |        |                                                                           |        |             |  |         |        |                                |        |                              |        |      |        |                               |        |  |  |

-continued

| Item                                                                      | Laydown g/m <sup>2</sup> |
|---------------------------------------------------------------------------|--------------------------|
| Layer 6 UV Overcoat                                                       |                          |
| Gelatin                                                                   | 0.8231                   |
| UV-1                                                                      | 0.0355                   |
| UV-2                                                                      | 0.2034                   |
| ST-4                                                                      | 0.0655                   |
| SF-1                                                                      | 0.0125                   |
| S-6                                                                       | 0.0797                   |
| 5-chloro-2-methyl-4-isothiazolin-3-one/2-methyl-4-isothiazolin-3-one(3/1) | 0.0001                   |
| Layer 7 SOC                                                               |                          |
| Gelatin                                                                   | 0.6456                   |
| Ludox AM™ (colloidal silica)                                              | 0.1614                   |
| Polydimethylsiloxane (DC200™)                                             | 0.0202                   |
| 5-chloro-2-methyl-4-isothiazolin-3-one/2-methyl-4-isothiazolin-3-one(3/1) | 0.0001                   |
| SF-2                                                                      | 0.0032                   |
| Tergitol 15-S-5™ (surfactant)                                             | 0.0020                   |
| SF-1                                                                      | 0.0081                   |
| Aerosol OT™ (surfactant)                                                  | 0.0029                   |

Coating format 1 was utilized to prepare the photographic print materials for the control. The control silver layers did not have the (i) and (ii) dopants and generally correspond to commercially available emulsions. None of the silver layers has (ii). The following imaging layers were coated utilizing curtain coating.

|         | Coating Format 1       | Laydown mg/m <sup>2</sup> |
|---------|------------------------|---------------------------|
| Layer 1 | Blue Sensitive Layer   |                           |
|         | Gelatin                | 1300                      |
|         | Blue sensitive silver  | 200                       |
|         | Y-1                    | 440                       |
|         | ST-23                  | 440                       |
|         | S-2                    | 190                       |
| Layer 2 | Interlayer             |                           |
|         | Gelatin                | 650                       |
|         | ST-4                   | 55                        |
|         | S-2                    | 160                       |
| Layer 3 | Green Sensitive        |                           |
|         | Gelatin                | 1100                      |
|         | Green sensitive silver | 70                        |
|         | M-1                    | 270                       |
|         | S-2                    | 75                        |
|         | S-3                    | 32                        |
|         | ST-8                   | 20                        |
|         | ST-21                  | 165                       |
|         | ST-22                  | 530                       |
| Layer 4 | UV Interlayer          |                           |
|         | Gelatin                | 635                       |
|         | UV-1                   | 30                        |
|         | UV-2                   | 160                       |
|         | ST-4                   | 50                        |
|         | S-10                   | 30                        |
|         | S-2                    | 30                        |
| Layer 5 | Red Sensitive Layer    |                           |
|         | Gelatin                | 1200                      |
|         | Red sensitive silver   | 170                       |
|         | C-1                    | 365                       |
|         | S-2                    | 360                       |
|         | UV-2                   | 235                       |
|         | S-9                    | 30                        |
|         | ST-4                   | 3                         |
| Layer 6 | UV Overcoat            |                           |
|         | Gelatin                | 440                       |
|         | UV-1                   | 20                        |
|         | UV-2                   | 110                       |
|         | ST-4                   | 30                        |

-continued

|    | Coating Format 1 | Laydown mg/m <sup>2</sup> |
|----|------------------|---------------------------|
| 5  | S-10             | 20                        |
|    | S-2              | 20                        |
|    | SOC              |                           |
| 10 | Gelatin          | 490                       |
|    | ST-4             | 17                        |
|    | SiO <sub>2</sub> | 200                       |
|    | Surfactant       | 2                         |
| 15 |                  |                           |
| 20 |                  |                           |

C-1



The D LogH characteristic curves were generated for the invention and control materials by electromodulated separation exposures (raster scanned) at 1000 nanoseconds. The 25 0.5 second exposures were made by contact printing using a carbon step tablet and separation filters. The 1000 ns digital exposures and the 0.5 second contact printed exposures were processed in conventional RA-4 development chemistry and read on a Status A reflection densitometer. 30 The separation curves were plotted, and shoulder density maximum and inmax values were taken from the plots. The FIGURE shows a D LogH characteristic curve. The Dmin value 10 is the intercept of the curve on the density axis, 12 is Dmax (maximum density), 14 is the speed point, 16 is the shoulder, and 18 is the inmax value. The distance between 35 10 and 0.04 units higher than 10 is indicated at 22. A % loss value was calculated for the shoulder, density maximum, and inmax. The % loss equation used was % loss = { (0.5 sec exposure value - 1000 ns exposure value) / 0.5 sec exposure 40 value } \* 100. The % loss values from the D LogH characteristic curves are listed in Table 1A below.

TABLE 1A

|    | Check % loss (0.5 secs vs 1000 ns) | Feature % loss (0.5 sec vs 1000 ns) |
|----|------------------------------------|-------------------------------------|
| 45 | Red Shoulder -37.3                 | -7.0                                |
|    | Green Shoulder -19.6               | -5.4                                |
| 50 | Blue Shoulder -27.8                | -2.3                                |
|    | Red Dmax -29.9                     | -3.4                                |
|    | Green Dmax -19.6                   | -6.4                                |
|    | Blue Dmax -16.9                    | -2.5                                |
|    | Red inmax -42.7                    | -6.7                                |
|    | Green inmax -23.3                  | -7.3                                |
| 55 | Blue inmax -33.1                   | -2.6                                |

The data from Table 1A clearly demonstrate the digital printing advantages that the invention has compared to the control. Since an ideal color paper would have a theoretical 60 % loss of zero across this extreme exposure range, a % loss of less than 10% in all color records is considered exceptional. For shoulder, Dmax, and inmax, the invention is clearly superior to the control color paper and is attributed to the significant and unexpected reciprocity control enabled 65 by the formulation of the invention. Because the color paper of the invention can be exposed over this extreme range of exposures (0.5 seconds to 1000 ns) with a % loss of less than

71

10% for each color record, the color paper of the invention has significant commercial value in that it can function in both a negative working optical exposure equipment and direct writing sub microsecond digital systems.

Model 16D. The output from this instrument is force, in millinewtons, required to bend the cantilevered, unclasped end of a sample 20 mm long and 38.1 mm wide at an angle of 15 degrees from the unloaded position. In this test the stiffness in both the machine direction and cross direction of the photographic element A and B was compared to the stiffness of typical low cost and premium photographic paper. L\* or lightness and opacity was measured for using a Spectrograph spectrophotometer, CIE system, using illuminant D6500. The test results for the above tests are listed in Table 3 below.

APPENDIX

S-1 = dibutyl phthalate



5  
10  
15

Y-1  
20  
25

SC-1  
30

M-1  
40  
45

ST-2

50  
55  
ST-3

60  
65  
ST-4

72

-continued

UV-1



UV-2



S-3 = 1, 4-Cyclohexyldimethylene bis(2-ethylhexanoate)

C-1



S-4 = 2-(2-Butoxyethoxy)ethyl acetate

Dye-1



The structure of photographic element of the invention (prior to overlamination with a polycarbonate sheet) was the following:

50 Coating Layers 1-7  
Top biaxially oriented, microvoided polyolefin sheet with TiO<sub>2</sub>, blue tint and optical brightener  
Ethylene plastomer with 10% anatase TiO<sub>2</sub>  
Cellulose paper base with 2% rutile TiO<sub>2</sub>, 254 micrometers thick and 0.10% blue dye  
Ethylene plastomer  
Bottom biaxially oriented polyolefin sheet  
sodium salt of styrene sulfonic acid  
60 The surface roughness of the emulsion side of each photographic element was measured by a Federal Profiler at three stages of sample preparation, in the paper base form, after extrusion lamination and after silver halide emulsion coating. The Federal Profiler instrument consists of a motorized drive nip which is tangent to the top surface of the base plate. The sample to be measured is placed on the base plate and fed through the nip. A micrometer assembly is sus-

pended above the base plate. The end of the spindle provides a reference surface from which the sample thickness can be measured. This flat surface is 0.95 cm diameter and, thus, bridges all fine roughness detail on the upper surface of the sample. Directly below the spindle, and nominally flush with the base plate surface, is a moving hemispherical stylus of the gauge head. This stylus responds to local surface variation as the sample is transported through the gauge. The stylus radius relates to the spatial content that can be sensed. The output of the gauge amplifier is digitized to 12 bits. The sample rate is 500 measurements per 2.5 cm. The thickness of the product was measured with a Mitutoyo digital linear gauge using a measurement probe head of 20 mm<sup>2</sup>. The test results for the above tests are listed in Table 3 below.

Sharpness, or the ability to replicate fine details of the image, was measured by mathematical calculations utilizing a method is called the MTF or Modulation Transfer Function. In this test, a fine repeating sinusoidal pattern of photographic density variation near the resolution of the human eye was exposed on a photographic print. When the image was developed, the resulting density variation was compared to the expected density, and a ratio was obtained to determine the magnitude of the transfer coefficient at that frequency. A number of 100 denotes perfect replication, and this number was relatively easy to obtain at spatial frequencies of 0.2 cycle/mm. At a finer spacing of 2.0 cycles/mm, typical color photographic prints have a 70 rating or 70% replication. The test results for the above tests are listed in Table 3 below.

Tear resistance for the photographic elements is the moment of force required to start a tear along an edge of the photographic element. The tear resistance test used was originally proposed by G. G. Gray and K. G. Dash, *Tappi Journal* 57, pages 167-170 published in 1974. The tear resistance for the photographic elements is determined by the tensile strength and the stretch of the photographic element. A 15 mm×25 mm sample is looped around a metal cylinder with a 2.5 cm diameter. The two ends of the sample are clamped by an Instron tensile tester. A load is applied to the sample at a rate of 2.5 cm per minute until a tear is observed, at which time the load, expressed in N, is recorded. The test results for the above tests are listed in Table 3 below.

The D LogH characteristic curves were generated for the invention and control materials by electromodulated separation exposures (raster scanned) at 125 nanoseconds. The exposures were processed in conventional RA-4 development chemistry and read on a Status A reflection densitometer. The curves were plotted, and density minimum (Dmin), low toe, and toe values were taken from the plots. The FIGURE shows a D LogH characteristic curve. The Dmin value 2 is the intercept of the curve on the density axis, 4 is the low toe value, 6 is the toe value, and 8 is the speed point. The values from the D LogH characteristic curves are listed in Table 4 below.

TABLE 3

| Performance Measure         | Control | Invention |
|-----------------------------|---------|-----------|
| MD Stiffness (millinewtons) | 173     | 370       |
| CD Stiffness (millinewtons) | 94      | 325       |
| L*                          | 93      | 95.3      |
| Opacity                     | 93      | 96.4      |
| MTF                         | 71      | 81        |
| Tear Strength (N)           | 129     | 707       |

TABLE 4

| 5       | Control |         |        | Invention |         |        |
|---------|---------|---------|--------|-----------|---------|--------|
|         | cyan    | magenta | yellow | cyan      | magenta | yellow |
| Dmin    | 0.106   | 0.094   | 0.106  | 0.095     | 0.079   | 0.092  |
| Low Toe | 0.203   | 0.195   | 0.180  | 0.184     | 0.182   | 0.169  |
| Toe     | 0.419   | 0.400   | 0.368  | 0.408     | 0.396   | 0.360  |

10 The data in Table 3 above comparing the invention to the control material show that the invention is clearly superior to the prior art photographic papers. The MD/CD stiffness for the invention is balanced; that is, the MD and CD stiffness are roughly equal creating a photographic image that is balanced in stiffness which is perceptually preferred over the control photographic paper which is much stronger in the machine direction compared to the cross direction. The tear resistance of the invention (707 N) is significantly improved over control material (129 N) resulting in improved image durability compared to prior art photographic color papers. The L\* and opacity for the invention is higher than that of the control leading to an image that is 15 brighter and has less show through compared to the control material. Image sharpness or the perceived clarity with which elements of an image are distinguished from one another was substantially improved over the control material. The invention MTF was 81 compared to a MTF of 71 20 for the control. A 10 unit increase in MFT is significant in that it reduces digital printing artifacts. The improvement in image sharpness for the invention is a function of higher weight percents of TiO<sub>2</sub> and the microvoided layer.

25 The data from Table 4 clearly demonstrate the digital printing advantages that the invention has compared to the control. The low toe values from the D LogH characteristic curves generated for the invention show a significant improvement compared to the control in the lower scale regions. The Dmin values for the invention improved by 10% for the cyan record, 16% for the magenta record, and 16% for the yellow record. As a result, it was found that the cyan low toe improved by 9%, the magenta low toe 30 improved by 7%, and the yellow low toe improved by 6% while maintaining an acceptable toe position. Since the Status A measurements include the base coloration (e.g., not density minimum corrected as would occur in typical print viewing), a significant portion of the low toe density measurement incorporates the Dmin. As density increases, this base Dmin contribution diminishes. The combination of the low toe improvement, lower density minimum for the invention compared to the control and a higher MTF for the invention yields as significant improvement in digital printing quality, minimizing many of the digital printing artifacts that occur in this region of the characteristic curve and that are typical for prior art photographic papers. This low toe 35 improvement and reduced minimum density served to reduce digital printing artifacts in digitally printed images. The improved Dmin for the invention also serves to increase the dye gamut of printed images. Finally, the reduction of digital printing artifacts combined with higher image sharpness, higher brightness, reduced Dmin, and improved image tear resistance yields an image that is superior to prior art photographic papers and thus has significant commercial 40 value.

The structure of photographic element of the invention (after overlamination with a polycarbonate sheet) was the following:

- Scratch resistant Polycarbonate sheet
- Adhesive layer
- Coating Layers 1-7
- Top biaxially oriented, microvoided polyolefin sheet with  $TiO_2$ , blue tint and optical brightener
- Ethylene plastomer with 10% anatase  $TiO_2$
- Cellulose paper base with 2% rutile  $TiO_2$ , 254 micrometers thick and 0.10% blue dye
- Ethylene plastomer
- Bottom biaxially oriented polyolefin sheet
- sodium salt of styrene sulfonic acid

TABLE 5

| Material             | Visible scratch |
|----------------------|-----------------|
| Polyethylene         | 2.0 grams       |
| Polypropylene        | 13.7 grams      |
| Polyester            | 18.7 grams      |
| Polycarbonate        | 22.5 grams      |
| Photographic Control | 2.0 grams       |

The scratch data in Table 5 clearly show that the photographic control polyethylene overlaminates are lower in scratch resistance than the polypropylene, polyester, and polycarbonate overlaminates. This data clearly demonstrate the need to provide scratch protection for a photographic surface particularly when they are to be used for displays. Photographic material may be repeatedly handled and precautions need to be taken. Polycarbonate is shown to be near 10 times more resistant to the formation of scratches than polyethylene, as well as more resistant than a typical photographic control which is hardened gelatin.

The scratch data was determined by applying a 1500 g ramped load force at a velocity of 10 mm/min. with a 54  $\mu m$  radius, 120 degree conical Rockwell Diamond stylus. The scratch length was 10 mm. The samples were then examined visually for the presence of a scratch.

The invention has been described in detail with particular reference to certain preferred embodiments thereof, but it will be understood that variations and modifications can be effected within the spirit and scope of the invention.

What is claimed is:

1. A photographic element comprising at least one photosensitive layer, and a base material comprising an upper and lower biaxially oriented polymer sheet separated by a paper sheet, wherein said base material has a thickness of greater than 254 micrometers, a stiffness of greater than 325 millinewtons in any direction, and an upper surface roughness of less than 0.45 micrometers at a spatial frequency of between 0.30 and 6.35 millimeters, and a transmission percent of less than 15 percent.

2. The photographic element of claim 1 wherein said paper sheet has a basis weight of greater than 200 g/m<sup>2</sup>.

3. The photographic element of claim 1 wherein said photographic element has a stiffness of between 325 and 650 millinewtons.

4. The photographic element of claim 1 wherein said photographic element has upper surface roughness of between 0.20 and 0.50 micrometers.

5. The photographic element of claim 1 wherein said paper sheet has a thickness of between 6.7 and 9.0 mils.

6. The photographic element of claim 1 wherein said photographic element has an exposure range of at least 125 nanoseconds to 0.5 seconds.

7. The photographic element of claim 1 wherein said base material comprising an upper and lower biaxially oriented polymer sheet separated by a paper sheet further comprises an adhesive layer between said upper and lower biaxially oriented polymer sheets and paper sheet.

8. The photographic element of claim 1 wherein said biaxially oriented polymer sheet further comprises at least one layer comprising voids.

9. The photographic element of claim 1 wherein said biaxially oriented polymer sheet further comprises at least one layer comprising white pigment.

10. A reflection display material comprising an image, a laminated base material, and a scratch resistant polymer sheet laminated onto the top surface of said image, wherein said laminated base material comprises an upper and lower biaxially oriented polymer sheet separated by a paper sheet, wherein said laminated base material has a thickness of greater than 254 micrometers, a stiffness of greater than 325 millinewtons in any direction, and an upper surface roughness of less than 0.45 micrometers at a spatial frequency of between 0.30 and 6.35 millimeters, and a transmission percent of less than 15 percent.

11. The reflection display material of claim 10 wherein said scratch resistant polymer sheet comprises a polycarbonate sheet.

12. The reflection display material of claim 10 wherein said scratch resistant polymer sheet has a scratch resistance of greater than 3 grams.

13. The reflection display material of claim 10 wherein said scratch resistant polymer sheet has a textured surface.

14. The reflection display material of claim 13 wherein said scratch resistant polymer sheet has a textured surface having a roughness average of 50 to 250 roughness average.

15. The reflection display material of claim 10 wherein said biaxially oriented polymer sheets comprise biaxially oriented polyolefin.

16. The reflection display material of claim 10 wherein said image comprises a photographic image.

17. The reflection display material of claim 10 wherein said scratch resistant polymer sheet comprises polyester, polyolefin, or polyamide.

18. A method of forming a reflection display material comprising providing a photographic element comprising at least one photosensitive layer, and a base material comprising an upper and lower biaxially oriented polymer sheet separated by a paper sheet, wherein said base material has a thickness of greater than 254 micrometers, a stiffness of greater than 325 millinewtons in any direction, and an upper surface roughness of less than 0.45 micrometers at a spatial frequency of between 0.30 and 6.35 millimeters, and a transmission percent of less than 15 percent, imaging said photographic element, developing said photographic element to produce an image, and bringing the developed photographic element into contact with a scratch resistant polymer sheet.